# EUROPEAN PATENT SPECIFICATION

(11) **EP 0 313 083 B1**
(45) Date of publication and mention of the grant of the patent: **10.01.1996**
(21) Application number: 88117593.9
(22) Date of filing: 21.10.1988
(51) Int. Cl.: G03C 7/32

(54) **Silver halide color photographic material**
Farbphotographisches Silberhalogenidmaterial
Matériau photographique couleur à l'halogénure d'argent

(30) Priority: 22.10.1987 JP 267478/87
(43) Date of publication of application: 26.04.1989
(73) Proprietor: FUJI PHOTO FILM CO., LTD., Kanagawa 250-01 (JP)
(72) Inventor: Mihayashi, Keiji c/o FUJI PHOTO FILM CO., LTD., Minami Ashigara-shi Kanagawa (JP); Kobayashi, Hidetoshi c/o FUJI PHOTO FILM CO., LTD., Minami Ashigara-shi Kanagawa (JP)
(74) Representative: Grünecker, Kinkeldey, Stockmair & Schwanhäusser Anwaltssozietät

(56) References cited:
- EP-A- 0 161 626
- EP-A- 0 226 849
- EP-A- 0 267 618
- PATENT ABSTRACTS OF JAPAN vol. 12, no. 25 (P-659)(2872), 26 January 1988; & JP-A- 62 180 365

## Description

The present invention refers to silver halide color photographic materials which contain naphthol based cyan couplers which have a substituent group in the 5-position and pyrazoloazole based magenta couplers which have an alkoxy group or an aryloxy group in the 6-position.

Good color forming properties, color reproduction and sharpness, good processing dependence, stability and colored image storage properties are desirable in silver halide color photosensitive materials. Naphthol based cyan couplers which satisfy the above mentioned requirements have been suggested in European Patent No. 161,626A, and magenta couplers have been suggested in U.S. Patent 4,540,654 and European Patent No. 226,849A. However, the use of either of these alone, results in only minimal improvement.

The combination of some of these couplers has been suggested in JP-A-62-180365 (the term "JP-A" as used herein signifies "unexamined published Japanese patent application"). The utilization of this combination results in an improvement of color reproduction, processing dependence and image storage properties. However, problems affecting photographic performance have arisen. These problems include instability of the silver halide photosensitive materials during storage.

EP-A-267618 which is comprised in the state of the art by virtue of Article 54(3) EPC discloses silver halide color photographic materials containing specific hydroquinone derivatives and pyrazoloazole and naphthol couplers wherein a two equivalent cyan coupler is incorporated into a red sensitive layer having the highest speed and a four equivalent coupler is incorporated into a red sensitive layer having the lowest speed.

It is the object of the present invention to provide a silver halide colour photographic material which has excellent colour reproduction, exhibits little variation in performance due to the passage of time during the storage of the coating liquids, during the manufacture of the sensitive material, during the storage of the photosensitive material, or during the storage of a latent image, in which the fluctuation in density after processing is slight even when deteriorated or low pH bleach or bleach-fix baths are used, and which exhibit sharpness at high speed.

Said object is achieved by a silver halide color photographic material comprising at least two red sensitive silver halide emulsion layers having different speeds and containing at least one cyan coupler; at least one green sensitive silver halide emulsion layer containing at least one magenta coupler; and at least one blue sensitive silver halide emulsion layer containing at least one yellow coupler, wherein said layers are established on a support and at least one of the cyan couplers is represented by the general formula (A), and at least one of the magenta couplers is represented by the general formula (I) or the general formula (II): wherein R₁ represents a halogen atom, an aliphatic group, an aromatic group, a heterocyclic group, an amidino group, a guanidino group or a group which is represented by -COR₄, -SO₂R₄, -SOR₄, -NHCOR₄, -NHSO₂R₄, -HNSOR₄, or R₂ represents a halogen atom, a hydroxyl group, a carboxyl group, a sulfo group, an amino group, a cyano group, a nitro group, an aliphatic group, an aromatic group, a carbonamido group, a sulfonamido group, a carbamoyl group, a sulfamoyl group, a ureido group, an acyl group, an acyloxy group, an aliphatic oxy group, an aromatic oxy group, an aliphatic thio group, an aromatic thio group, an aliphatic sulfonyl group, an aromatic sulfonyl group, an aliphatic sulfinyl group, an aromatic sulfinyl group, an aliphatic oxycarbonyl group, an aromatic oxycarbonyl group, an aliphatic oxycarbonylamino group, an aromatic oxycarbonylamino group, a sulfamoylamino group, a heterocyclic group or an imido group,
ℓ' is 0 or an integer of up to 3, R₃ represents a hydrogen atom or a R₆U group, T represents a hydrogen atom or a group which can be eliminated by a coupling reaction with the oxidized form of a primary aromatic amine developing agent; R₄ and R₅ each independently represent an aliphatic group, an aromatic group, a heterocyclic group, an amino group, an aliphatic oxy group or an aromatic oxy group, R₆ represents a hydrogen atom, an aliphatic group, an aromatic group, a heterocyclic group,
a -OR₇, a -SR₇ group, a -COR₈ group, a group, a -PO(R₇)₂ group, a -PO(-OR₇)₂ group, a group, a SO₂N a -CO₂R₇ group, a -SO₂R₇ group, a -SO₂OR₇ group or an imido group, and U represents a group, a -CO- group, a -SO₂- group, a -SO- group or a single bond, R₇ represents an aliphatic group, an aromatic group or a heterocyclic group, R₈ represents a hydrogen atom, an aliphatic group, an aromatic group or a heterocyclic group and R₉ and R₁₀ each independently represent a hydrogen atom, an aliphatic group, an aromatic group, a heterocyclic group, an acyl group, an aliphatic sulfonyl group or an aromatic sulfonyl group or may be joined together to form a ring, when ℓ' has a value of 2 or more, the R₂ groups may be the same or different, or they may be joined together to form a ring or R₂ and R₃, or R₃ and T, may be joined together to form rings, respectively ; or dimers or larger units (oligomers or polymers) can be formed by linking together via divalent groups or groups of higher valence in any of R₁, R₂, R₃ or T; with the proviso that said cyan coupler of formula (A) is not
wherein R₃₁ represents an alkyl group, an aryl group or a heterocyclic group,
R₃₂ represents a hydrogen atom or a substituent group, R_{32'} represents an alkyl group, an aryl group, an alkylthio group, an arylthio group or a heterocyclic thio group, and
X represents a hydrogen atom or a coupling elimination group,
wherein the red sensitive layer having the lowest speed contains a four equivalent cyan coupler of the general formula (A) wherein T is a hydrogen atom and the red sensitive layer having the highest speed contains a two equivalent cyan coupler of the general formula (A) wherein T is a group other than a hydrogen atom.

Compounds which can be used in the invention are described below.

The term "aliphatic groups signifies a linear chain, branched or cyclic alkyl group, alkenyl group or alkynyl group, and these may be substituted or unsubstituted groups. The term "aromatic group" signifies a substituted or unsubstituted aryl group and these may have condensed rings. The term "heterocyclic group" signifies a substituted or unsubstituted, simple ring or condensed ring, heterocyclic group.

Actual examples of aliphatic groups include a methyl group, ethyl group, n-propyl group, i-propyl group, n-butyl group, i-butyl group, t-butyl group, cyclopentyl group, t-pentyl group, cyclohexyl group, n-octyl group, 2-ethylhexyl group, n-decyl group, ndodecyl group, n-tetradecyl group, n-hexadecyl group, noctadecyl group, 2-hexyldecyl group, adamantyl group, trifluoromethyl group, carboxymethyl group, methoxyethyl group, vinyl group, allyl group, hydroxyethyl group, heptafluoropropyl group, benzyl group, phenethyl group, phenoxyethyl group, methylsulfonylethyl group, methylsulfonamidoethyl group, 3-(2-ethylhexyloxy)propyl group, 3-n-decyloxypropyl group, 3-n-dodecyloxypropyl group, 3n-tetradecyloxypropyl group, oleyl group, propargyl group, ethenyl group, 3-(2,4-di-t-pentylphenoxy)propyl group, 4-(2,4-di-t-pentylphenoxy)butyl group, 1-(2,4-dit-pentylphenoxy)propyl group, 1-(2,4-di-t-pentylphenoxy)pentyl group, 1-(3-tetradecylphenoxy)propyl group, and 2-n-dodecylthioethyl group.

Actual examples of aromatic groups include a phenyl group, p-tolyl group, m-tolyl group, o-tolyl group, 4-chlorophenyl group, 4-nitrophenyl group, 4-cyanophenyl group, 4-hydroxyphenyl group, 3-hydroxy-phenyl group, 1-naphthyl group, 2-naphthyl group, o-biphenylyl group, p-biphenylyl group, pentafluorophenyl group, 2-methoxyphenyl group, 2-ethoxyphenyl group, 4-methoxyphenyl group, 4-t-butylphenyl group, 4-t-octylphenyl group, 4-carboxyphenyl group, 4-methylsulfonamidophenyl group, 4-(4-hydroxyphenylsulfonyl)phenyl group, 2-n-tetradecyloxyphenyl group, 4-n-tetradecyloxyphenyl group, 2-chloro-5-n-dodecyloxyphenyl group, 3n-pentadecylphenyl group, 2-chlorophenyl group, 4-methoxycarbonylphenyl group, 4-methylsulfonylphenyl group, and 2,4-di-t-pentylphenyl group.

Actual examples of heterocyclic groups include a 2-pyridyl group, 3-pyridyl group, 4-pyridyl group, 2-furyl group, 2-thienyl group, 3-thienyl group, 4-quinolyl group, 2-imidazolyl group, 2-benzimidazolyl group, 4-pyrazolyl group, 2-benzo-oxazolyl group, 2-benzthiazolyl group, 1-imidazolyl group, 1-pyrazolyl group, 5-tetrazolyl group, 1,3,4-thiadiazol-2-yl group, 2-pyrrolyl group, 3-triazolyl group, 4-oxazolyl group, 4-thiazolyl group, 2-pyrimidyl group, 1,3,5-triazin-2-yl group, 1,3,4-oxadiazol-2-yl group, 5-pyrazolyl group, 4-pyrimidyl group, 2-pyrazyl group, succinimido group, phthalimido group, morpholino group, pyrrolidino group, piperidino group, imidazolidin-2,4-dione-3-yl group, imidazolidin-2,4-dione-1-yl group, and oxazolidin-2,4dione-3-yl group.

The individual substituent groups in the general formula [A] are described in detail below.

R₁ in general formula [A] represents a halogen atom, aliphatic group, aromatic group, heterocyclic group, amidino group, guanidino group or a group which can be represented by -COR₄, -SO₂R₄, -SOR₄, -NHCOR₄, -NHSO₂R₄, -NHSOR₄ or R₄ and R₅ each independently represent an aliphatic group which preferably has from 1 to 30 carbon atoms, an aromatic group which preferably has from 6 to 30 carbon atoms, a heterocyclic group which preferably has from 1 to 30 carbon atoms, an amino group which preferably has from 0 to 30 carbon atoms [for example an amino group, methylamino group, dimethylamino group, n-butylamino group, anilino group, N-(2-n-tetradecyloxyphenyl)amino group, pyrrolidino group, morpholino group, piperidino group, 2-ethylhexylamino group, n-dodecylamino group, N-methyl-N-dodecylamino group, 3-dodecyloxypropylamino group, 3-(2,4-di-t-pentylphenoxy)propylamino group, 4-(2,4-di-t-pentylphenoxy)butylamino group], an aliphatic oxy group which preferably has from 1 to 30 carbon atoms [for example a methoxy group, ethoxy group, butoxy group, methoxyethoxy group, n-dodecyloxy group, 3-(2,4-di-t-pentylphenoxy)propoxy group] or an aromatic oxy group which preferably has from 6 to 30 carbon atoms [for example a phenoxy group, 4-n-dodecyloxyphenoxy group, 4-methoxycarbonylphenoxy group]. R₄ and R₅ may also be joined together to form a ring. When R₁ is a halogen atom this halogen atom can be a fluorine atom, chlorine atom, bromine atom or iodine atom. When R₁ is an amidino group or guanidino group the group preferably has from 1 to 30 carbon atoms and may be substituted with aliphatic groups, aromatic groups, hydroxyl groups, aliphatic oxy groups, acyl groups, aliphatic sulfonyl groups, aromatic sulfonyl groups, acyloxy groups, aliphatic sulfonyloxy groups or aromatic sulfonyloxy groups. Further, two nitrogen atoms may be joined together to form a heterocycle such as an imidazole or a benzimidazole.

R₂ in general formula [A] represents a halogen atom (fluorine atom, chlorine atom, bromine atom or iodine atom), hydroxyl group, carboxyl group, sulfo group, cyano group, nitro group, an amino group which preferably has from 0 to 30 carbon atoms (for example an amino group, methylamino group, dimethylamino group, pyrrolidino group, anilino group), an aliphatic group which preferably has from 1 to 30 carbon atoms, an aromatic group which preferably has from 6 to 30 carbon atoms, a carbonamido group which preferably has from 1 to 30 carbon atoms (for example formamido group, acetamido group, trifluoroacetamido group, benzamido group), a sulfonamido group which preferably has from 1 to 30 carbon atoms (for example methylsulfonamido group, trifluoromethylsulfonamido group, n-butylsulfonamido group, p-tolylsulfonamido group), a carbamoyl group which preferably has from 1 to 30 carbon atoms (for example carbamoyl group, N,N-dimethylcarbamoyl group, N-methylcarbamoyl group, pyrrolidinocarbonyl group, N-n-hexadecylcarbamoyl group), a sulfamoyl group which preferably has from 0 to 30 carbon atoms (for example sulfamoyl group, N-methylsulfamoyl group, N,N-dimethylsulfamoyl group, morpholinosulfonyl group, N-n-dodecylsulfamoyl group), a ureido group which preferably has from 1 to 30 carbon atoms (for example ureido group, 3-methylureido group, 3-phenylureido group, 3,3-dimethylureido group), an acyl group which preferably has from 1 to 30 carbon atoms (for example acetyl group, pivaloyl group, benzoyl group, dodecanoyl group), an acyloxy group which preferably has from 1 to 30 carbon atoms (for example acetoxy group, benzoyloxy group), an aliphatic oxy group which preferably has from 1 to 30 carbon atoms, an aromatic oxy group which preferably has from 6 to 30 carbon atoms, an aliphatic thio group which preferably has from 1 to 30 carbon atoms, an aromatic thio group which preferably has from 6 to 30 carbon atoms, an aliphatic sulfonyl group which preferably has from 1 to 30 carbon atoms, an aromatic sulfonyl group which preferably has from 6 to 30 carbon atoms, an aliphatic sulfinyl group which preferably has from 1 to 30 carbon atoms, an aromatic sulfinyl group which preferably has from 6 to 30 carbon atoms, an aliphatic oxycarbonyl group which preferably has from 2 to 30 carbon atoms, an aromatic oxycarbonyl group which has preferably from 7 to 30 carbon atoms, an aliphatic oxycarbonylamino group which preferably has from 2 to 30 carbon atoms, an aromatic oxycarbonylamino group which preferably has from 7 to 30 carbon atoms, a sulfamoylamino group which preferably has from 0 to 30 carbon atoms (for example sulfamoylamino group, 3,3-dimethylsulfamoylamino group, piperidinosulfonylamino group), a heterocyclic group which preferably has from 1 to 30 carbon atoms or an imido group which preferably has from 4 to 30 carbon atoms (for example a succinimido group, maleimido group, phthalimido group, diglycolimido group, 4-nitrophthalimido group).

R₃ in general formula [A] represents a hydrogen atom or R₆U. Here R₆ represents a hydrogen atom, an aliphatic group which preferably has from 1 to 30 carbon atoms, an aromatic group which preferably has from 6 to 30 carbon atoms, a heterocyclic group which preferably has from 1 to 30 carbon atoms, an -OR₇ group, an SR₇ group, a -COR₈ group, an group, a -PO(R₇)₂ group, a -PO(-OR₇)₂ group, a group, an group, a -CO₂R₇ group, an -SO₂R₇ group, an -SO₂OR₇ group, or an imido group which preferably has from 4 to 30 carbon atoms (for example succinimido group, maleimido group, phthalimido group, diacylamino group). U represents an 〉N-R₉ group, -CO- group, -SO₂- group, -SO- group or a single bond. R₇ represents an aliphatic group which preferably has from 1 to 30 carbon atoms, an aromatic group which preferably has from 6 to 30 carbon atoms or a heterocyclic group which preferably has from 1 to 30 carbon atoms. R₈ represents a hydrogen atom, an aliphatic group which preferably has from 1 to 30 carbon atoms, an aromatic group which preferably has from 6 to 30 carbon atoms or a heterocyclic group which preferably has from 1 to 30 carbon atoms. R₉ and R₁₀ each independently represents a hydrogen atom, an aliphatic group which preferably has from 1 to 30 carbon atoms, an aromatic group which preferably gas from 6 to 30 carbon atoms, a heterocyclic group which preferably has from 1 to 30 carbon atoms, an acyl group which preferably has from 1 to 30 carbon atoms (for example acetyl group, trifluoroacetyl group, benzoyl group, p-chlorobenzoyl group) or a sulfonyl group which preferably has from 1 to 30 carbon atoms (for example methylsulfonyl group, n-butylsulfonyl group, phenylsulfonyl group, p-nitrophenylsulfonyl group). R₉ and R₁₀ may be joined together to form a ring.

T in general formula [A] represents a hydrogen atom or a group which can be eliminated by a coupling reaction with the oxidized form of a primary aromatic amine developing agent. Examples of the latter type of group include halogen atoms (fluorine atom, chlorine atom, bromine atom and iodine atom), sulfo group, thiocyanato group, isothiocyanato group, selenocyanato group, aliphatic oxy groups which preferably have from 1 to 30 carbon atoms, aromatic oxy groups which preferably have from 6 to 30 carbon atoms, aliphatic thio groups which preferably have from 1 to 30 carbon atoms, aromatic thio groups which preferably have from 6 to 30 carbon atoms, heterocyclic thio groups which preferably have from 1 to 30 carbon atoms, heterocyclic oxy groups which preferably have from 1 to 30 carbon atoms, aromatic azo groups which preferably have from 6 to 30 carbon atoms, heterocyclic groups which preferably have from 1 to 30 carbon atoms, acyloxy groups which preferably have from 1 to 30 carbon atoms (for example acetoxy group, benzoyloxy group), sulfonyloxy groups which preferably have from 1 to 30 carbon atoms (for example methylsulfonyloxy group, p-tolylsulfonyloxy group), carbamoyloxy groups which preferably have from 1 to 30 carbon atoms (for example N,N-dimethylcarbamoyloxy group, pyrrolidinocarbonyloxy group, N-ethylcarbamoyloxy group), thiocarbonyloxy groups which preferably have from 2 to 30 carbon atoms (for example methylthiocarbonyloxy group, phenylthiocarbonyloxy group), and carbonyldioxy groups which preferably from 2 to 30 carbon atoms (for example methoxycarbonyloxy group, phenoxycarbonyloxy group).

R₂ and R₃, R₃ and T, or a plurality of R₂ groups in general formula [A] may be joined together to form rings respectively. Examples of cases in which R₂ and R₃ are joined together include the -CH₂CO- group, -OCOgroup, -NHCO- group, -C(CH₃)₂CO- group and the -CH=CHCO group. Examples of cases in which R₃ and T are joined together include the -CH₂C- group and the -COO- group. Examples of cases in which a plurality of R₂ groups are joined together include the -(CH₂)₃- group, -(CH₂)₄ group, -OCO- group, -OCONH- group, -NHCONH- group, -(CH=CH)₂- group, -OCH₂O- group, -OCH₂CH₂O- group, and the -OC(CH₃)₂O- group.

Examples of preferred substituent groups for the compounds represented by the general formula [A] are described below.

R₁ in general formula [A] is preferably a halogen atom, a -COR₄ group or an -SO₂R₄ group, and cases in which R₄ is an amino group are especially desirable. Examples of the -COR₄ group include a carbamoyl group, Nethylcarbamoyl group, N-n-butylcarbamoyl group, N-cyclohexylcarbamoyl group, N-(2-ethylhexyl)carbamoyl group, N-dodecylcarbamoyl group, N-hexadecylcarbamoyl group, N-(3-decyloxypropyl)carbamoyl group, N-(3-dodecyloxypropyl)carbamoyl group, N-[3-(2,4-di-t-pentylphenoxy)propyl]carbamoyl group, N-[4-(2,4-di-t-pentylphenoxy)butyl]carbamoyl group, N,N-dimethylcarbamoyl group, N,N-dibutylcarbamoyl group, N-methyl-N-dodecylcarbamoyl group, morpholinocarbamoyl group, N-methyl-N-phenylcarbamoyl group, N-(2-tetradecyloxyphenyl)carbamoyl group, N-phenylcarbamoyl group, N-(4-tetradecyloxyphenyl)carbamoyl group, N-(2-propoxyphenyl)carbamoyl group, N-(2-chloro-5-dodecyloxyphenyl)carbamoyl group, N-(2-chlorophenyl)carbamoyl group. Examples of the - SO₂R₄ group include a sulfamoyl group, N-methylsulfamoyl group, N,N-diethylsulfamoyl group, N,N-diisopropylsulfamoyl group, N-(3-dodecyloxypropyl)sulfamoyl group, N-[3-(2,4-di-t-pentylphenoxy)propyl]sulfamoyl group, N-[4-(2,4-di-t-pentylphenoxy)butyl]sulfamoyl group, pyrrolidinosulfamoyl group, N-phenylsulfamoyl group, N-(2-butoxyphenyl)sulfamoyl group, N-(2-tetradecyloxyphenyl)sulfamoyl group. R₁ is most desirably a -COR4 group (R₄ being an amino group).

(R₂)ℓ ´ in general formula [A] is preferably such that ℓ ´ is zero, followed by the case in which e' is equal to 1. When ℓ'=1, the R₂ group is preferably a halogen atom, aliphatic group, aromatic oxy group, carbonamido group, sulfonamido group, or cyan group. Of these groups the most desirable are a fluorine atom, chlorine atom, trifluoromethyl group, methoxy group and a cyano group. The R₂ group is preferably substituted in the 2-position or the 4-position with respect to the R₃NH- group.

In R₃ in general formula [A], R₆ is preferably an aliphatic group, aromatic group, -OR₇ group or an -SR₇ group, and U is preferably -CO- or -SO₂-. Examples of aliphatic groups include a methyl group, trifluoromethyl group, trichloromethyl group, ethyl group, heptafluoroethyl group, t-butyl group, 1-ethylpentyl group, cyclohexyl group, benzyl group, undecenyl group, tridecenyl group, and 1-(2,4-di-t-pentylphenoxy)propyl group. Examples of aromatic groups include a phenyl group, 1-naphthyl group, 2-naphtyl group, 2-chlorophenyl group, 4-methoxyphenyl group, 4-nitrophenyl group, and pentafluorophenyl group. Examples of -OR₇ groups include a methoxy group, isopropoxy group, n-butoxy group, iso-butoxy group, t-butoxy group, n-pentyloxy group, n-hexyloxy group, n-octyloxy group, 2-ethylhexyl group, n-decyloxy group, n-dodecyloxy group, 2-methoxyethoxy group, benzyloxy group, trichloroethoxy group, trifluoroethoxy group, phenoxy group, and p-methylphenoxy group. Examples of -SR₇ groups include a methylthio group, ethylthio group, allylthio group, n-butylthio group, benzylthio group, n-dodecylthio group, phenylthio group, p-t-octylphenylthio group, p-dodecylphenylthio group, and a p-octyloxyphenylthio group. More desirably, R₃ is an aliphatic oxycarbonyl group (R₆ is R₇O- and U is -CO-) or an aliphatic or aromatic sulfonyl group (R₆ is an aliphatic group or an aromatic group and U is -SO₂) and, most desirably, R₃ is an aliphatic oxycarbonyl group.

T in general formula [A] is preferably a hydrogen atom, halogen atom, aliphatic oxy group, aromatic oxy group, aliphatic thio group or a heterocyclic thio group. Examples of the aliphatic oxy groups include a methoxy group, ethoxy group, 2-hydroxyethoxy group, 2-chloroethoxy group, carboxymethoxy group, 1-carboxyethoxy group, methoxyethoxy group, 2-(2-hydroxyethoxy)ethoxy group, 2-methyl-sulfonylethoxy group, 2-methylsulfonyloxyethoxy group, 2-methylsulfonylamidoethyl group, 2-carboxyethoxy group, 3-carboxypropoxy group, 2-(carboxymethylthio)ethoxy group, 2-(1-carboxytridecylthio)ethoxy group, 1-carboxytridecyl group, N-(2-methoxyethyl)carbamoylmethoxy group, 1-imidazolylmethoxy group, and a 5-phenoxycarbonylbenzotriazol-1-ylmethoxy group. Examples of aromatic oxy groups include a 4-nitrophenoxy group, 4-acetamidophenoxy group, 2-acetamidophenoxy group, 4-methylsulfonylphenoxy group, and a 4-(3-carboxypropanamido)phenoxy group. Examples of the aliphatic thio group include a methylthio group, 2-hydroxyethylthio group, carboxymethylthio group, 2-carboxyethylthio group, 1-carboxyethylthio group, 3-carboxypropylthio group, 2-dimethylaminoethylthio group, benzylthio group, n-dodecylthio group, and a 1-carboxytridecylthio group. Examples of heterocyclic thio groups include a 1-phenyl-1,2,3,4-tetrazol-5-ylthio group, 1-ethyl-1,2,3,4-tetrazol-5-ylthio group, 1-(4-hydroxyphenyl)-1,2,3,4-tetrazol-5-ylthio group, 4-phenyl-1,2,4-triazol-3-ylthio group, 5-methyl-1,3,4-oxadiazol-2-ylthio group, 1-(2-carboxyethyl)-1,2,3,4-tetrazol-5-ylthio group, 5-methylthio-1,3,4-thiadiazol-2-ylthio group, 5-methyl-1,3,4-thiadiazol-2-ylthio group, 5-phenyl-1,3,4-oxadiazol-2-ylthio group, 5-amino-1,3,4-thiadiazol-2-ylthio group, benzoxazol-2-ylthio group, 1-methylbenzimidazol2-ylthio group, 1-(2-dimethylaminophenyl)-1,2,3,4-tetrazol-5-ylthio group, benzothiazol-2-ylthio group, 5-(ethoxycarbonylmethylthio)-1,3,4-thiadiazol-2-ylthio group, 1,2,4-triazol-3-ylthio group, 4-pyridylthio group, and a 2-pyrimidylthio group. More desirably, T is a hydrogen atom, chlorine atom, aliphatic oxy group or an aliphatic thio group, and most desirably T is a hydrogen atom or an aliphatic oxy group.

Couplers which can be represented by the general formula [A] may take the form of dimers or larger units which are bonded together via divalent groups or groups of higher valency in the substituent groups R₁, R₂, R₃ or T. In such cases the number of carbon atoms may be outside the specified range for each of the aforementioned types of substituent groups.

Typical examples of cases in which the couplers represented by the general formula [A] are in an oligomeric form include homopolymers or copolymers of addition polymerizable ethylenically saturated compounds which have cyan dye forming coupler residual groups (cyan color forming monomers). In this case the oligomer has repeating units of general formula [B], and, one or more types of the cyan color forming repeating units represented by the general formula [B] can be included in the oligomer, or the oligomer may take the form of a copolymer which contains one or more non-color forming ethylenic monomers as a copolymerized component.

In this formula R represents a hydrogen atom, an alkyl group which has from 1 to 4 carbon atoms or a chlorine atom. G represents a -CONH- group, a -COO-group or a substituted or unsubstituted phenylene group. J represents a substituted or unsubstituted alkylene group, phenylene group or aralkylene group. L represents a -CONH- group, -NHCONH- group, -NHCOO-group, -NHCO- group, -OCONH- group, -NH- group, -COO-group, -OCO- group, -CO- group, -O- group, -SO₂- group, -NHSO₂- group or an -SO₂NH- group. Moreover, a', b' and c' each represent 0 or 1. Q represents a cyan coupler residual group in which a hydrogen atom other than that of the hydroxyl group in the 1-position has been removed from a compound which can be represented by the general formula [A].

Copolymers of cyan color forming monomers which provide a coupler unit of general formula [B] and the non-color forming ethylenic monomers indicated below are preferred as oligomers.

Non-color forming ethylenic monomers which do not couple with the oxidation products of primary aromatic amine developing agents include acrylic acid, α-chloroacrylic acid, α-alkylacrylic acids (for example methacrylic acid), esters and amides derived from these acrylic acids (for example acrylamide, methacrylamide, n-butylacrylamide, t-butylacrylamide, diacetoneacrylamide, N-methylolacrylamide, N-(1,1-dimethyl-2-sulfonatoethyl)acrylamide, N-(3-sulfonatopropyl)acrylamide, methyl acrylate, ethyl acrylate, n-propyl acrylate, n-butyl acrylate, t-butyl acrylate, isobutyl acrylate, acetoacetoxyethyl acrylate, n-hexyl acrylate, 2-ethylhexyl acrylate, n-octyl acrylate, lauryl acrylate, methyl methacrylate, ethyl methacrylate, n-butyl methacrylate, and β-hydroxyethylmethacrylate), vinyl esters (for example vinyl acetate, vinyl propionate and vinyl laurate), acrylonitrile, methacrylonitrile, aromatic vinyl compounds (for example styrene and derivatives thereof, such as vinyltoluene, divinyl benzene, potassium styrenesulfinate, vinylacetophenone and sulfostyrene), itaconic acid, citraconic acid, crotonic acid, vinylidene chloride, vinyl alkyl ethers, (for example vinyl ethyl ether), maleic acid esters, N-vinyl-2-pyrrolidone, N-vinylpyridine and 2- and 4-vinylpyridine.

The acrylic acid esters, methacrylic acid esters and maleic acid esters are especially desirable. Two or more types of the non-color forming ethylenic monomers can be used together. For example, it is possible to use methyl acrylate and butyl acrylate, butyl acrylate and styrene, butyl methacrylate and methacrylic acid, methyl acrylate and diacetoneacrylamide, N-(1,1-dimethyl-2-sulfonatoethyl)acrylamide and acrylic acid, or potassium styrenesulfinate and N-vinylpyrrolidone.

The ethylenic unsaturated monomer for copolymerization with a vinyl based monomer corresponding to the aforementioned general formula [B] is selected so as to improve the physical and/or chemical properties of the copolymer which is formed, as is well known in the polymeric coupler field. For example, these properties include solubility, compatibility with binding agents such as gelatin used in photographic colloid compositions, flexibility and heat resistance.

The selection of a lipophilic non-color forming ethylenic monomer (for example an acrylic acid ester, methacrylic acid ester, maleic acid ester, vinyl benzene) as the principal copolymer component is preferred for obtaining lipophilic polymeric couplers which are soluble in organic solvents.

The lipophilic polymeric couplers obtained by the polymerization of a vinyl monomer provide a coupler unit which can be represented by the aforementioned general formula [B]. [B] can be made by emulsification and dispersion in the form of a latex in aqueous gelatin solution, or by direct emulsion polymerization.

Methods for the emulsification and dispersion of lipophilic polymeric couplers in the form of a latex in aqueous gelatin solution are disclosed in U.S. Patent 3,451,820. Methods for emulsion polymerization are disclosed in U.S. Patents 4,080,211 and 3,370,952.

The use of hydrophilic non-color forming ethylenic monomers such as N-(1,1-diethyl-2-sulfonatoethyl)acrylamide, 3-sulfonatopropyl acrylate, sodium styrenesulfonate, potassium 2-styrenesulfinate, acrylamide, methacrylamide, acrylic acid, methacrylic acid, N-vinylpyrrolidone, N-vinyl pyridine for the copolymer component is preferred for obtaining hydrophilic polymeric couplers which can be dissolved in neutral or alkaline water.

Hydrophilic polymeric couplers can be added to coating liquids as aqueous solutions, and they can also be added as solutions in solvent mixtures obtained by mixing water with a lower alcohol, tetrahydrofuran, acetone, ethyl acetate, cyclohexane, ethyl lactate, dimethylformamide, or dimethylacetamide. Moreover, they can be added after being dissolved in aqueous alkaline solutions and alkali containing organic solvents. A small quantity of surfactant can also be added.

Actual examples of couplers represented by the general formula [A] which can be used in the invention are indicated below,

In general formula (I) R₃₁ represents an alkyl group, aryl group or a heterocyclic group, and R₃₂ represents a hydrogen atom or a substituent group. X represents a hydrogen atom or a coupling elimination group.

In general formula (II) R₃₁ represents the same groups as mentioned above. R₃₂' represents an alkyl group, alkylthio group, arylthio group, heterocyclic thio group or an aryl group. X represents a hydrogen atom or a coupling elimination group.

More precisely, R₃₁ represents an alkyl group such as a methyl group, ethyl group, isopropyl group, t-butyl group, trifluoromethyl group, phenylmethyl group, methoxyethyl group, 2-phenoxyethyl group, 2-methylsulfonylethyl group, 2-hydroxyethyl group, 3,3,3-trifluoropropyl group, 2-fluoroethyl group, 2-chloroethyl group, 2-bromoethyl group, 2-cyanoethyl group, 3-oxobutyl group or an aryl group such as a phenyl group, 4-methylphenyl group, 4-t-butylphenyl group, 4-acylaminophenyl group, 4-halogenophenyl group, 4-alkoxyphenyl group, or a heterocyclic group such as a 2-furyl group, 2-thienyl group, 2-pyrimidyl group, 2-benzothiazolyl group, 2-pyridyl group, 3-pyridyl group, and a 4-pyridyl group. Of these, preferred examples for R₃₁ include methyl group, ethyl group, isopropyl group, t-butyl group, methoxyethyl group and 2-phenoxyethyl group.

R₃₂ is a hydrogen atom, a halogen atom (for example a chlorine atom, bromine atom), an alkyl group [for example a substituted alkyl group such as a sulfonamido substituted alkyl group (e.g., sulfonamidomethyl group, 1-sulfonamidoethyl group, 2-sulfonamidoethyl group, 1-methyl-2-sulfonamidoethyl group, 3-sulfonamidopropyl group), acylamino substituted alkyl group (e.g., acylaminomethyl group, 1-acylaminoethyl group, 2-acylaminoethyl group, 1-methyl-2-acylaminoethyl group, 3-acylaminopropyl group), sulfonamido substituted phenylalkyl group (e.g., p-sulfonamidophenylmethyl group, p-sulfonamidophenylethyl group, 1-(p-sulfonamidophenyl)ethyl group, p-sulfonamidophenylpropyl group), acylamino substituted phenylalkyl group (e.g., p-acylaminophenylmethyl group, p-acylaminophenylethyl group, 1-(p-acylminophenyl)ethyl group, p-acylaminophenylpropyl group), alkylsulfonyl substituted alkyl group (e.g., 2-dodecylsulfonylethyl group, 1-methyl-2-pentadecylsulfonylethyl group, octadecylsulfonylpropyl group), phenylsulfonyl substituted alkyl group (e.g., 3-(2-butyl-5-t-octylphenylsulfonyl)propyl group, 2-(4-dodecyloxyphenylsulfonyl)ethyl group), or an unsubstituted alkyl group such as a methyl group, ethyl group, hexyl group, dodecyl group], an aryl group (for example a substituted aryl group such as a sulfonamidophenyl group, acylaminophenyl group, alkoxyphenyl group, aryloxyphenyl group, substituted alkylphenyl group, sulfonamidonaphthyl group, acylaminonapthyl group or an unsubstituted aryl group such as a phenyl group, naphthyl group), a heterocyclic group (for example a 2-furyl group, 2-thienyl group, 2-pyrimidinyl group, 2-benzothiazolyl group), a cyano group, an alkoxy group (for example a methoxy group, ethoxy group, 2-methoxyethoxy group, 2-dodecylethoxy group, 2-methanesulfonylethoxy group), an aryloxy group (for example a phenoxy group, 2-methylphenoxy group, 4-t-butylphenoxy group), an acylamino group (for example an acetamido group, benzamido group, tetradecanamido group, α-(2,4-di-t-amylphenoxy)butylamido group, γ-(3-t-butyl-4-hydroxyphenoxy)butylamide group, α-[4-(4-hydroxyphenylsulfonylphenoxy)decanamido group), an anilino group (for example a phenylamino group, 2-chloroanilino group, 2-chloro-5tetradecanamidoanilino group, 2-chloro-5-dodecyloxy-carbonylanilino group, N-acetylanilino group, 2-chloro-5-[α-(3-t-butyl-4-hydroxyphenoxy)dodecanamido]anilino group), a ureido group (for example a phenylureido group, methylureido group, N,N-dibutylureido group), a sulfamoylamino group (for example an N,N-dipropylsulfamoylamino group, N-methyl-N-decylsulfamoylamino group), an alkylthio group (for example a methylthio group, octylthio group, tetradecylthio group, 2-phenoxyethylthio group, 3-phenoxypropylthio group, 3-(4-t-butylphenoxy)propylthio group), an arylthio group (for example a phenylthio group, 2-butoxy-5-t-octylphenylthio group, 3-pentadecylphenylthio group, 2-carboxyphenylthio group, 4-tetradecanamidophenylthio group), an alkoxycarbonylamino group (for example a methoxycarbonylamino group, tetradecyloxycarbonylamino group), a sulfonamido group (for example a methanesulfonamido group, hexadecanesulfonamido group, benzenesulfonamido group, p-toluenesulfonamido group, octadecanesulfonamido group, 2-methyloxy-5-butylbenzenesulfonamido group), a carbamoyl group (for example an N-ethylcarbamoyl group, N,N-dibutylcarbamoyl group, N-(2-dodecyloxyethyl)carbamoyl group, N-methyl-N-dodecylcarbamoyl group, N-[3-(2,4-di-t-amylphenoxy)propyl]carbamoyl group), a sulfamoyl group (for example an N-ethylsulfamoyl group, N,N-dipropylsulfamoyl group, N-(2-dodecyloxyethyl)sulfamoyl group, N-ethyl-N-dodecylsulfamoyl group, N,N-diethylsulfamoyl group), a sulfonyl group (for example a methanesulfonyl group, octanesulfonyl group, benzenesulfonyl group, toluenesulfonyl group), or an alkoxycarbonyl group (for example a methoxycarbonyl group, butyloxycarbonyl group, dodecyloxycarbonyl group, octadecyloxycarbonyl group). Of these groups the alkyl groups, aryl groups, alkylthio groups and arylthio groups are preferred, and the alkyl groups and aryl groups are the more desirable.

R₃₂' represents a substituted alkyl group, such as a sulfonamido substituted alkyl group (for example a sulfonamidomethyl group, 1-sulfonamidoethyl group, 2-sulfonamidoethyl group, 1-methyl-2-sulfonamidoethyl group, 3-sulfonamidopropyl group), an acylamino substituted alkyl group (for example an acylaminomethyl group, 1-acylaminoethyl group, 2-acylaminoethyl group, 1-methyl-2-acylaminoethyl group, 3-acylaminopropyl group), a sulfonamido substituted phenylalkyl group (for example a p-sulfonamidophenylmethyl group, p-sulfonamidophenylethyl group, 1-(p-sulfonamidophenyl)ethyl group, p-sulfonamidophenylpropyl group), an acylamino substituted phenylalkyl group (for example p-acylaminophenylmethyl group, p-acylaminophenylethyl group, 1-(p-acylaminophenyl)ethyl group, p-acylaminophenylpropyl group), an alkylsulfonyl substituted alkyl group (for example a 2-dodecylsulfonylethyl group, 1-methyl-2-pentadecylsulfonylethyl group, octadecylsulfonylpropyl group), a phenylsulfonyl substituted alkyl group (e.g., 3-(2-butyl-5-t-octylphenylsulfonyl)propyl group, 2-(4-dodecyloxyphenylsulfonyl)ethyl group), or an unsubstituted alkyl group such as a methyl group, ethyl group, hexyl group, dodecyl group, a substituted aryl group such as a sulfonamidophenyl group, acylaminophenyl group, alkoxyphenyl group, aryloxyphenyl group, substituted alkylphenyl group, sulfonamidonaphthyl group, acylaminonaphthyl group, or an unsubstituted aryl group such as a phenyl group, naphthyl group, or an alkylthio group (for examples a methylthio group, octylthio group, tetradecylthio group, 2-phenoxyethylthio group, 3-phenoxypropylthio group, 3-(4-t-butylphenoxy)propylthio group), an arylthio group (for example a phenylthio group, 2-butoxy-5-t-octylphenylthio group, 3-pentadecylphenylthio group, 2-carboxyphenylthio group, 4-tetradecanamidophenylthio group), or a heterocyclic thio group (for example a 2-benzothiazolylthio group, 2,4-diphenoxy-1,3,5-triazol-6-thio group, 2-pyridylthio group).

Of these groups the substituted alkyl groups and substituted aryl groups are preferred, and the substituted alkyl groups are the more desirable.

X represents, for example, a hydrogen atom, halogen atom (for example chlorine atom, bromine atom, or iodine atom), carboxyl group or a group which is linked via an oxygen atom (for example acetoxy group, propanoyloxy group, benzoyloxy group, 2,4-dichlorobenzoyloxy group, ethoxyoxaloyloxy group, pyruvinyloxy group, cinnamoyloxy group, phenoxy group, 4-cyanophenoxy group, 4-methanesulfonamidophenoxy group, 4-methanesulfonylphenoxy group, α-naphthoxy group, 3-pentadecylphenoxy group, benzyloxycarbonyloxy group, ethoxy group, 2-cyanoethoxy group, benzyloxy group, 2-phenethyloxy group, 2-phenoxyethoxy group, 5-phenyltetrazolyloxy group, 2-benzothiazolyloxy group), a group which is linked via a nitrogen atom (for example benzenesulfonamido group, N-ethyltoluenesulfonamido group, heptafluorobutanamido group), 2,3,4,5,6-pentafluorobenzamido group, octanesulfonamido group), p-cyanophenylureido group, N,N-diethylsulfamoylamino group, 1-piperidyl group, 5,5-dimethyl-2,4-dioxo-3-oxazolidinyl group, 1-benzylethoxy-3-hydantoinyl group, 2N-1,1-dioxo-3(2H)-oxo-1,2-benzoisothiazolyl group, 2-oxo-1,2-dihydroxy-1-pyridinyl group, imidazolyl group, pyrazolyl group, 3,5-diethyl-1,2,4-triazol-1-yl group, 5- or 6-bromobenzotriazol-1-yl group, 5-methyl-1,2,3,4-tetrazol-l-yl group, benzimidazolyl group), or a group which is linked via a sulfur atom (for example phenylthio group, 2-carboxyphenylthio group, 2-methoxy-5-t-octylphenylthio group, 4-methanesulfonylphenylthio group, 4-octanesulfonamidophenylthio group, benzylthio group, 2-cyanoethylthio group, l-ethoxycarbonyltridecylthio group, 5-phenyl-2,3,4,5-tetrazolylthio group, 2-benzothiazolyl group). Of these, preferred examples for X include chlorine atom, an aryloxy group (e.g., phenoxy group, 4-cyanophenoxy group, 4-methanesulfonamidophenoxy group, 4-methanesulfonylphenoxy group), and an arylthio group (e.g., phenylthio group, 2-methoxy-5-t-octylphenylthio group, 2-butoxy-5-t-octylphenylthio group).

In cases where R₃₁, R₃₂, R₃₂' or X is a divalent linking.group and dimers are formed, R₃₁, R₃₂ or R₃₂' represents a substituted or unsubstituted alkylene group (for example methylene group, ethylene group, 1,10-decylene group, -CH₂CH₂-O-CH₂-CH₂- group), a substituted or unsubstituted phenylene group (for example 1,4-phenylene group, 1,3-phenylene group, and X represents a divalent group corresponding appropriately with the above mentioned univalent groups.

The linking groups represented by any of R₃₁, R₃₂ or R₃₂' when the compounds represented by the general formulae [I] and [II] are included in a vinyl monomer are groups established by combining groups selected from among the alkylene groups (substituted or unsubstituted alkylene groups, for example methylene group, ethylene group, 1,10-decylene group, -CH₂CH₂OCH₂CH₂- group), phenylene groups (substituted and unsubstituted phenylene groups, for example 1,4-phenylene group, 1,3-phenylene group -NHCO- group, -CONH- group, -O- group, -OCO- group and the aralkylene groups (for example

The preferred linking groups are indicated below: -CH₂CH₂-, -CH₂CH2NHCO-, -CH₂CH₂O-CH₂CH₂-NHCO-,

Moreover, the vinyl group may have substituent groups other than that represented by the general formula [I] and the preferred substituent groups are hydrogen atoms, chlorine atoms and lower alkyl groups which have from 1 to 4 carbon atoms (for example methyl group, ethyl group).

Monomers which contain a part which can be represented by general formula [I] or general formula [II] can be formed into copolymers with non-color forming ethylenic monomers which do not couple with the oxidation products of primary aromatic amine developing agents.

Examples of non-color forming ethylenic monomers which do not couple with the oxidation products of primary aromatic amine developing agents include acrylic acid, α-chloroacrylic acid, α-alkylacrylic acids (for example methacrylic acid), esters and amides derived from these acrylic acids (for example acrylamide, methacrylamide, n-butylacrylamide, t-butylacrylamide, diacetoneacrylamide, methacrylamide, methyl acrylate, ethyl acrylate, n-propyl acrylate, n-butyl acrylate, t-butyl acrylate, isobutyl acrylate, 2-ethylhexyl acrylate, n-octyl acrylate, lauryl acrylate, methyl methacrylate, ethyl methacrylate, n-butyl methacrylate and β-hydroxyethylmethacrylate), methylenebisacrylamide, vinyl esters (for example vinyl acetate, vinyl propionate and vinyl laurate), acrylonitrile, methacrylonitrile, aromatic vinyl compounds (for example styrene and derivatives thereof, vinyltoluene, divinyl benzene, vinylacetophenone and sulfostyrene), itaconic acid, citraconic acid, crotonic acid, vinylidene chloride, vinyl alkyl ethers (for example vinyl ethyl ether), maleic acid, maleic anhydride, maleic acid esters, N-vinyl-2-pyrrolidone, N-vinylpyridine and 2-and 4-vinylpyridine. Two or more types of non-color forming ethylenic monomer used here can be used together. For example, it is possible to use n-butyl acrylate and methyl methacrylate, styrene and methacrylic acid, methacrylic acid and acrylamide, or methyl acrylate and diacetoneacrylamide.

The non-color forming ethylenically unsaturated monomer for copolymerization with a solid water insoluble monomeric coupler is selected so as to improve the physical and/or chemical properties of the copolymer which is formed, as is well known in the polymeric field. For example, these properties include solubility, compatibility with binding agents such as gelatin used in photographic colloid compositions, flexibility and heat resistance.

The polymeric couplers used in the present invention may be water soluble or water insoluble. The use of polymeric coupler latexes from these materials is preferred.

Actual examples of typical magenta couplers to be used in this invention are indicated below.

The cyan couplers represented by the general formula [A] can be easily prepared using the method disclosed in European Patent No. 161,626A. Furthermore, the magenta couplers represented by the general formulae [I] and [II] can be easily prepared using the methods disclosed in European Patent No. 226,849A and U.S. Patent 4,540,654.

The cyan couplers represented by the general formula [A] are added to a red sensitive emulsion layer and/or adjacent layers. and the total amount added is usually from 0.01 to 1.5 g/m, preferably from 1.0 to 1.2 g/m, and more desirably from 0.2 to 1.0 g/m.

The red sensitive emulsion layer consists of two or more layers which have different speeds.

A four equivalent cyan coupler wherein T is a hydrogen atom is used in the layer having the lowest speed and a two equivalent coupler wherein T is a group other than a hydrogen atom is used in the layer having the highest speed.

The method used to add the cyan couplers to the photosensitive material is based on the method used for the other couplers described hereinafter. However, the amount of high boiling point organic solvent which is used as a dispersing medium with respect to the couplers is preferably from 0 to 1.0, more desirably from 0 to 0.5, and most desirably from 0 to 0.3, in terms of the ratio by weight.

The magenta couplers represented by general formula [I] or [II] are added to the green sensitive emulsion layer and/or adjacent layers, and the total amount added is usually from 0.01 to 1.0 g/m, preferably from 0.05 to 0.8 g/m, and more desirably from 0.1 to 0.5g/m,

The method used to add the magenta couplers to the photosensitive material is based on the method used for the other couplers described hereinafter. However, the amount of high boiling point organic solvent which is used as a dispersing medium with respect to the couplers is from 0 to 4.0, preferably from 0.1 to 2.0, and more desirably from 0.3 to 1.0, in terms of the ratio by weight.

In the photographic material of this invention, at least one blue-sensitive layer, at least one green-sensitive layer and at least two red-sensitive layers are coated on a support. There are no restrictions with respect to the order and the number of the silver halide emulsion layer and the non light-sensitive layer. As a typical example, there is a silver halide photographic material comprising a light-sensitive layer consisting of a plurality of silver halide emulsion layers which have substantially the same color sensitivity but a different light sensitivity, wherein a unit light-sensitive layer has a sensitivity with respect to any one of blue light, green light, or red light. Furthermore, in a multilayer silver halide color photographic material, the order of a unit light-sensitive layer is generally a red-sensitive layer, a green-sensitive layer, and a blue-sensitive layer from the support. According to the purpose, this coating order may be in reverse order, or a layer having a different light sensitivity may be inserted into a layer having the same color sensitivity.

Various types of a non light-sensitive layer such as an intermediate layer may be coated between the silver halide light-sensitive layers, and . may be used as an uppermost layer or a lowermost layer.

The intermediate layer may contain a coupler described in JP-A-61-43748, JP-A-59-113438, JP-A-59-113440, JP-A-61-20037, and JP-A-200381 or a DIR coupler or a color-mixing preventing agent as in a conventional photographic material.

The plural silver halide layers which constitute the unit light-sensitive layer are preferably, comprised of two layers having a high sensitive emulsion layer and a low sensitive emulsion layer as disclosed in West German Patent 1,121,470 and British Patent 923,045 Usually, the preferred order is such that the light sensitivity of the silver halide layers decreases orderly towards the support, and a non light-sensitive may be coated between each silver halide emulsion layer. Moreover, as disclosed in JP-A-57-112751, JP-A-62-200350, JP-A-62-206541, and JP-A-62-206543, a low-sensitive layer may be coated on the farther side from the support and a high-sensitive emulsion layer may be coated in the nearer side from the support.

As an illustrative example, there are, from the farthest side from a support, a low-sensitive blue-sensitive layer (BL)/a high-sensitive blue-sensitive layer (BH)/a high-sensitive green-sensitive layer (GH)/a low-sensitive green-sensitive layer (GL)/a high-sensitive red-sensitive layer (RH)/a low-sensitive red-sensitive layer (RL), BH/BL/GL/GH/RH/RL or BH/BL/GH/GL/RL/RH.

As disclosed in JP-B-55-34932 (the term "JP-B" as used herein means an "examined Japanese patent publication"), the order of a blue-sensitive layer/GH/RH/GL/RL from the farthest side from a support may be used. Moreover, as disclosed in JP-A-56-25738 and JP-A-62-63936, the order of a blue-sensitive layer/GL/RL/GH/RH from the farthest side from a support may be used.

As disclosed in JP-B-49-15495, the arrangement having the constitution of three layers differing in light sensitivity in which a silver halide emulsion layer having the highest light sensitivity is used as an upper layer, a silver halide emulsion layer having a lower light sensitivity than that of the upper layer is used as a middle layer, and a silver halide emulsion layer having a lower light sensitivity than that of the middle layer is used as a lower layer and the light sensitivity of the silver halide emulsion layers decreases orderly towards the support may be used. Even when such a structure having three layers differing in light-sensitivity is used, the order of a middle-sensitive emulsion layer/a high-sensitive emulsion layer/a low-sensitive emulsion layer from the farthest side from a support may be used in a same color sensitivity layer as described in JP-A-59-202464.

As described above, various types of a layer structure and a layer order can be selected according to the purpose of the photographic materials.

The silver halide contained in the photographic emulsions of the photographic materials of the present invention, is preferably a silver iodobromide, silver iodochloride or silver iodochlorobromide which contains not more than about 30 mol% of silver iodide. The most desirable silver halides are silver iodobromides which contain from about 2 mol% to about 25 mol% of silver iodide.

The silver halide grains in the photographic emulsion may have a regular crystalline form, such as a cubic form, an octahedral form or a tetradecahedral form, an irregular crystalline form such as a spherical form or a tabular from, a form in which there are crystal defects such as twinned crystal planes, or forms in which these various forms are combined.

The grain size of the silver halide may be fine with a grain diameter of less than about 0.2 µm or large with a projected area diameter up to about 10 µm. Further, the grains may take the form of a poly-disperse emulsion or a mono-disperse emulsion.

The silver halide photographic emulsion used in the present invention can be prepared utilizing known methods including those disclosed on pages 22 to 23 of Research Disclosure (RD) No. 17643 (February 1978), "I, Emulsion Preparation and Types", in RD No. 18716 (November 1979), page 648; in Chemie et Physique Photographique, by P. Glafkides, published by Paul Montel, 1967; in Photographic Emulsion Chemistry, by G.F. Duffin, published by Focal Press, 1966; and in Making and Coating Photographic Emulsions, by V.L. Zelikman et al., published by Focal Press, 1964.

The mono-disperse emulsions disclosed in U.S. Patents 3,574,628 and 3,655,394 and British Patent 1,413,748 are preferred.

Furthermore tabular grains which have an aspect ratio of at least about 5 can be used in the present invention. Tabular grains can be easily prepared utilizing known methods including those disclosed by Gutoff in Photographic Science and Engineering, Volume 14, pp. 248 - 257 (1970), in U.S. Patents 4,434,226, 4,414,310, 4,433,048 and 4,439,520, and in British Patent 2,112,157.

The crystal structure of the grains may be uniform, the interior and exterior parts may have a heterogeneous halogen composition or the grains may have a layered structure. Further, silver halides of different compositions may be joined with an epitaxial junction or they may be joined to compounds other than silver halides such as silver thiocyanate or lead oxide.

Mixtures of grains of various crystalline forms may also be used.

The silver halide emulsions used are normally subjected to physical ripening, chemical ripening and spectral sensitization. Additives which can be used in these processes have been disclosed in Research Disclosure Nos. 17643 and 18716 and the locations of these items are summarized in the table below.

Known photographically useful additives which can be used in the present invention are also disclosed in the two Research Disclosures mentioned above and the locations of these disclosures are also shown in the table below.

| | Kind of Additives | RD 17643 | RD 18716 |
|---|---|---|---|
| 1. | Chemical sensitizers | Page 23 | Page 648, right column |
| 2. | Speed increasing agents | | as above |
| 3. | Spectral sensitizers and supersensitizers | Pages 23 to 24 | Page 648, right column to page 649, right column |
| 4. | Whiteners | Page 24 | |
| 5. | Anti-foggants and stabilizers | Pages 24 to 25 | Page 649, right column |
| 6. | Light absobers, filter dyes and UV absorbers | Pages 25 to 26 | Page 649, right column to page 650, left column |
| 7. | Anti-staining agents | Page 25, right column | Page 650, left column to right column |
| 8. | Dye image stabilizers | Page 25 | |
| 9. | Film hardening agents | Page 26 | Page 651, left column |
| 10. | Binders | Page 26 | as above |
| 11. | Plasticizers and lubricants | Page 27 | Page 650, right column |
| 12. | Coating promoters, surfactants | Pages 26 to 27 | as above |
| 13. | Anti-static agents | Page 27 | as above |

Various color couplers can be used additionally in this invention, and examples of these are disclosed in the patents discussed in Research Disclosure (RD) No. 17643, VII-C to G.

The use of the yellow color couplers of U.S. Patents 3,933,501, 4,022,620, 4,326,024 and 4,401,752, JP-B-58-10739, and British Patents 1,425,020 and 1,476,760 is preferred.

The 5-pyrazolone based and pyrazoloazole based compounds are preferred as magenta couplers. The magenta couplers disclosed in U.S. Patents 4,310,619 and 4,351,897, European Patent 73,636, U.S. Patents 3,061,432 and 3,725,067, Research Disclosure No. 24220 (June 1984), JP-A-60-33552, Research Disclosure No. 24230 (June 1984), JP-A-60-43659, and in U.S. Patents 4,500,630 and 4,540,654 are most desirable.

Phenol based and naphthol based couplers are used as cyan couplers, and those disclosed in U.S. Patents 4,052,212, 4,146,396, 4,228,233, 4,296,200, 2,369,929, 2,801,171, 2,772,162, 2,895,826, 3,772,002, 3,758,308, 4,334,011 and 4,327,173, West German Patent Application (OLS) No. 3,329,729, European Patent 121,365A, and in U.S. Patents 3,446,622, 4,333,999, 4,451,559 and 4,427,767 are preferred.

The colored couplers for correcting unwanted absorptions of the colored dyes disclosed in Research Disclosure No. 17643, section VII-G, U.S. Patent 4,163,670, JP-B-57-39413, U.S. Patents 4,004,929 and 4,138,258, and in British Patent 1,146,368 are preferred.

Couplers whose colored dyes have a suitable degree of diffusibility such as those disclosed in U.S. Patent 4,366,237, British Patent 2,125,570, European Patent 96,570, and in West German Patent Application (OLS) No. 3,234,533 are preferred.

Typical examples of polymerized dye forming couplers have been disclosed in U.S. Patents 3,451,820, 4,080,211 and 4,367,282, and in British Patent 2,102,173.

Couplers that release residual groups and are useful photographically in coupling, are also desirable for use in the present invention. The use of the DIR couplers which release development inhibitors disclosed in the patents indicated in the aforementioned Research Disclosure No. 17643, section VII-F, in JP-A-57-151944, JP-A-57-254234 and JP-A-60-184248, and in U.S. Patent 4,248,962 is desirable.

The use of couplers, which release nucleating agents or development accelerators in the form of the image during development, disclosed in British Patents 2,097,140 and 2,131,188, and in JP-A-59-157638 and JP-A-59-170840 is desirable.

Other couplers which can be used in the photosensitive materials of the present invention include the competitive couplers disclosed in U.S. Patent 4,130,427, the multi-equivalent couplers disclosed in U.S. Patents 4,283,472, 4,338,393 and 4,310,618, the DIR redox compound releasing couplers disclosed in JP-A-60-185950, the couplers which release a dye which restores coloration after elimination disclosed in European Patent 173,302A, the bleach accelerator releasing couplers disclosed in Research Disclosure No. 11449 and 24241, and in JP-A-61-201247, and the ligand releasing couplers disclosed in U.S. Patent 4,553,477.

The couplers which are used in the present invention can be introduced into the light sensitive materials by various known methods of dispersion.

Examples of high boiling point solvents which can be used in the oil in water dispersion methods have been disclosed in U.S. Patent 2,322,027.

Examples of the latex dispersion method and of latexes for impregnation purposes have been disclosed in U.S. Patent 4,199,363 and in West German Patent Application (OLS) Nos. 2,541,274 and 2,541,230.

Suitable supports which can be used in the present invention have been disclosed on page 28 of the aforementioned Research Disclosure No. 17643, and in the section from the right hand column of page 647 to the left hand column of page 648 of Research Disclosure No. 18716.

In the photographic material of the present invention, it is preferred that the total film thickness of the hydrophilic colloid layer is 28 µm or less in the side of the emulsion layer and that the film swelling speed (T_{1/2}) is 30 s or less. The film thickness means a film thickness which is determined under moisture conditioning at 25°C for 55% RH (2 days). The film swelling speed (T_{1/2}) is determined according to a known method in the art, for example, using a swelling meter whose type is described in A. Green et al, Photographic Science and Engineering, vol. 19, No. 2, pages 124 to 129. The film swelling speed (T_{1/2}) is defined as the time in which the film thickness reaches a saturated film thickness which is 90% of the maximum swell thickness when treated with a color developer at 30°C for 3 min and 15 s.

The film swelling speed (T_{1/2}) can be adjusted by adding a hardener to gelatin as a binder or changing the conditions with time after coating. Furthermore, the swell (%) is preferably 150 to 400%. The swell (%) is calculated from the following equation using a maximum swell film thickness in the above condition:$\text{Swell (%) =} \frac{\left(\text{Maximum swell film thickness -Film thickness}\right)}{\text{Film thickness}} \text{× 100}$

The color development bath used, is preferably an aqueous alkaline solution which contains a primary aromatic amine based color developing agent as the principal component. Aminophenol based compounds are useful as color developing agents. The use of p-phenylenediamine based compounds is preferred. Typical examples of these compounds include 3-methyl-4-amino-N,N-diethylaniline, 3-methyl-4-amino-N-ethyl-N-β-hydroxyethylaniline, 3-methyl-4-amino-N-ethyl-N-β-methanesulfonamidoethylaniline, 3-methyl-4-amino-N-ethyl-N-β-methoxyethylaniline, and the sulfate, hydrochloride and p-toluenesulfonate salts of these compounds. Two or more of these compounds can be used conjointly, depending on the intended purpose.

The color development baths generally contain pH buffers such as the carbonates, borates or phosphates of alkali metals, and development inhibitors or antifogging agents such as bromides, iodides, benzimidazoles, benzothiazoles or mercapto compounds. They may also contain, as required, various preservatives, such as hydroxylamine, diethylhydroxylamine, sulfite, hydrazines, phenylsemicarbazides, triethanolamine, catechol sulfonic acids, triethylenediamine (1,4-diazabicyclo[2,2,2]octane), organic solvents such as ethylene glycol and diethylene glycol, development accelerators such as benzyl alcohol, poly(ethylene glycol), quaternary ammonium salts and amines, color forming couplers, competitive couplers, fogging agents such as sodium borohydride, auxiliary developing agents such as l-phenyl-3-pyrazolidone, viscosity imparting agents, various chelating agents as typified by the aminopolycarboxylic acids, aminopolyphosphonic acids, alkylphosphonic acids and phosphonocarboxylic acids, typical examples of which include ethylenediamine tetraacetic acid, nitrilotriacetic acid, diethylenetriamine pentaacetic acid, cylohexanediamine tetraacetic acid, hydroxyethylimino diacetic acid, 1-hydroxyethylidene-1,1-diphosphonic acid, nitrilo-N,N,N-trimethylenephosphonic acid, ethylenediamine-N,N,N',N'-tetramethylenephosphonic acid, ethylenediamine di(o-hydroxyphenylacetic acid), and salts of these compounds.

Color development is carried out after a normal black and white development in the case of reversal processing. The known black and white developing agents, for example the dihydroxybenzenes such as hydroquinone, the 3-pyrazolidones such as 1-phenyl-3-pyrazolidone, and the amino phenols such as N-methyl-p-aminophenol, can be used individually or in combinations in the black and white development bath.

The pH of the color and black and white developing baths is generally within the range of from 9 to 12. Furthermore, the replenishment rate of the development bath depends on the color photographic material which is being processed, but it is generally less than 3 l/m of photosensitive material and it is possible, by reducing the bromide ion concentration in the replenisher, to use a replenishment rate of less than 500 ml/m of photosensitive material. The prevention of evaporation, and aerial oxidation, by minimizing the contact area with the air in the processing tank is desirable in cases where the replenishment rate is low. Furthermore, the replenishment rate can be reduced by suppressing the accumulation of bromide ion in the developer.

The photographic emulsion layers are subjected to a normal bleaching process after color development. The bleaching process may be carried out at the same time as the fixing process (in a bleach-fix process) or it may be carried out as a separate process. Moreover, a bleach-fix process can be carried out after a bleach process in order to speed-up processing. Also, processing can be carried out in two connected bleach-fix baths, a fixing process can be carried out before carrying out a bleach-fix process, or a bleaching process can be carried out after a bleach-fix process, according to the intended purpose of the processing. Compounds of a multivalent metal such as iron(III), cobalt(III), chromium(VI), copper(II), peracids, quinones, nitro compounds can be used as bleaching agents. Typical bleaching agents include ferricyanides; dichromates; organic complex salts of iron(III) or cobalt(III). Examples of complex salts with aminopolycarboxylic acids include ethylenediamine tetraacetic acid, diethylenetriamine pentaacetic acid, cyclohexanediamine tetraacetic acid, methylimino diacetic acid, 1,3-diaminopropane tetraacetic acid, glycol ether diamine tetraacetic acid or citric acid, tartaric acid or malic acid; persulfates; bromates; permanganates and nitrobenzenes. Of these materials the use of the aminopolycarboxylic acid iron(III) complex salts, principally ethylenediamine tetraacetic acid iron(III) complex salts, and persulfates, is preferred from the points of view of both rapid processing and the prevention of environmental pollution. Moreover, the amino polycarboxylic acid iron(III) complex salts are especially useful in both bleach baths and bleach-fix baths. The pH of the bleach or bleach-fix baths in which aminopolycarboxylic acid iron(III) complex salts are being used is normally from 5.5 to 8, but processing can be carried out at lower pH values to speed-up processing.

Bleach accelerators can be used, as required, in the bleach baths, bleach-fix baths, or bleach or bleach-fix pre-baths. Actual examples of useful bleach accelerators have been disclosed in the following specifications: compounds having a mercapto group or a disulfide group are disclosed in U.S. Patent 3,893,858, West German Patents 1,290,812 and 2,059,988, JP-A-53-32736, JP-A-53-57831, JP-A-53-37418, JP-A-53-72623, JP-A-53-95630, JP-A-53-95631, JP-A-53-104232, JP-A-53-124424, JP-A-53-141623 and JP-A-53-28426, and in Research Disclosure No. 17129 (July 1978); the thiazolidine derivatives disclosed in JP-A-50-140129; the thiourea derivatives disclosed in JP-B-45-8506, JP-A-50-20832 and JP-A-53-32735, and U.S. Patent 3,706,561; the iodides disclosed in West German Patent 1,127,715 and in JP-A-58-16235; the polyoxyethylene compounds disclosed in West German Patents 966,410 and 2,748,430; the polyamine compounds disclosed in JP-B-55-8836; the other compounds disclosed in JP-A-49-42434, JP-A-49-59644, JP-A-53-94927, JP-A-54-35727, JP-A-55-26506, and JP-A-58-163940; and bromide ions. Among these compounds, those which have a mercapto group or a disulfide group are preferred in view of their large acceleration effect, and the use of the compounds disclosed in U.S. Patent 3,893,858, West German Patent 1,290,812 and JP-A-53-95630 is especially desirable. Moreover, the use of the compounds disclosed in U.S. Patent 4,552,834 is also desirable. These bleach accelerators may be added to the sensitive material. These bleach accelerators are especially effective when bleach-fixing color photosensitive materials for photographic purposes.

Thiosulfates, thiocyanates, thioether based compounds, thioureas and large quantities of iodides can be used as fixing agents, but thiosulfates are generally used for this purpose, and ammonium thiosulfate in particular can be used in the widest range of applications. Sulfites or bisulfites, or carbonyl-bisulfite addition compounds, are the preferred preservatives for bleach-fix baths.

The silver halide color photographic materials of this invention are generally subjected to a water washing and/or stabilizing process after the desilvering process. The amount of water used in the water washing process can be fixed within a wide range according to the nature of the photosensitive material (for example the materials, such as the couplers, which are being used), the purpose for use, the wash water temperature, the number of washing tanks (the number of washing stages), the replenishment system, i.e., whether a counter-flow or a sequential-flow system is used, and various other conditions. The relationship between the amount of water used and the number of water washing tanks in a multi-stage counter-flow system can be obtained using the method outlined on pages 248 to 253 of Journal of the Society of Motion Picture and Television Engineers, Volume 64 (May 1955).

The amount of wash water can be greatly reduced by using the multi-stage counter-flow system noted in the aforementioned literature, but bacteria proliferate due to the increased residence time of the water in the tanks, thus causing sediments to form on the photosensitive material. A method to reduce calcium ion and manganese ion concentrations is disclosed in JP-A-62-288838. This method can be used very effectively to overcome problems of sedimentation in the processing of color photosensitive materials of the present invention. Furthermore, the isothiazolone compounds and thiabendazoles disclosed in JP-A-57-8542, and the chlorine based disinfectants such as chlorinated sodium isocyanurate, and benzotriazoles, and the disinfectants disclosed in Chemistry of Biocides and Fugicides by Horiguchi, Reduction of Microorganisms, Biocidal and Fungicidal Techniques, published by the Health and Hygiene Technical Society and in A Dictionary of Biocides and Fungicides, published by the Japanese Biocide and Fungicide Society, can be used for this purpose.

The pH of the wash water used in the processing of the photosensitive materials of the invention is within the range of from 4 to 9, and preferably within the range of from 5 to 8. The wash water temperature and washing time can be set variously according to the nature of the photosensitive material and the application. In general, washing conditions of from 20 seconds to 10 minutes at a temperature of from 15 to 45°C, and preferably of from 30 seconds to 5 minutes at a temperature of from 25 to 40°C, are selected. Moreover, the photosensitive materials of the present invention can be processed directly in a stabilizing bath instead of being subjected to a water wash as described above. The known methods disclosed in JP-A-57-8543, JP-A-58-14834 and JP-A-60-220345 can all be used for this purpose.

Furthermore, a stabilization process may be carried out following the aforementioned water washing process. The stabilizing baths contain formalin and surfactant and are used as a final bath for color photosensitive materials. Various chelating agents and fungicides can be added to these stabilizing baths.

The overflow which accompanies replenishment of the above mentioned wash water and/or stabilizer can be re-used in other processes such as a desilvering process.

A color developing agent may also be incorporated into the silver halide color photosensitive materials of the present invention in order to simplify and speed-up processing. The use of various color developing agent precursors is preferred for incorporation. For example, the indoaniline based compounds disclosed in U.S. Patent 3,342,597, the Schiff's base type compounds disclosed in U.S. Patent 3,342,599 and in Research Disclosure Nos. 14850 and 15159, the aldol compounds disclosed in Research Disclosure No. 13924, the metal salt complexes disclosed in U.S. Patent 3,719,492, and the urethane based compounds disclosed in JP-A-53-135628 can be used for this purpose.

Various 1-phenyl-3-pyrazolidones can be incorporated, as required, into the silver halide color photosensitive materials of this invention with a view to accelerating color development. Typical compounds of this type have been disclosed in JP-A-56-64339, JP-A-57-144547 and JP-A-58-115438.

The various processing baths are used at a temperature of from 10 to 50°C in the present invention. The standard temperature is normally from 33 to 38°C, but processing is accelerated and the processing time is shortened at higher temperatures and, conversely, higher picture quality and improved stability of the processing baths can be achieved at lower temperatures. Furthermore, processes using hydrogen peroxide intensification or cobalt intensification as disclosed in West German Patent 2,226,770 or U.S. Patent 3,674,499 can be carried out in order to economize on silver in the photosensitive material.

Furthermore, the silver halide photosensitive materials of this invention can also be used as heat developable photosensitive materials as disclosed in U.S. Patent 4,500,626, JP-A-60-133449, JP-A-59-218443 and JP-A-61-238056, and in European Patent 210,660A2.

The following examples further illustrate the present invention.

### COMPARATIVE EXAMPLE 1

Sample 101, a multi-layer color photosensitive material, was prepared by the lamination coating of each of the layers on an undercoated cellulose triacetate film support. The composition of the layers is indicated below.

### (Photosensitive Layer Compositions)

The numbers corresponding to each component indicate the amount coated onto the support, in units of grams per square meter, the amount after calculation as silver being shown in the case of the silver halides and colloidal silver. In the case of the sensitizing dyes, the amount coated is indicated in units of mols per mol of silver halide in the same layer.

### Sample 101

### First Layer (Anti-halation Layer)

| | |
|---|---|
| Black colloidal silver | as silver 0.18 |
| Gelatin | 0.40 |

### Second Layer (Intermediate Layer)

### Third Layer (First Red Sensitive Emulsion Layer)

| | |
|---|---|
| Mono-disperse silver iodobromide emulsion (6 mol% AgI, Average grain size 0.6 µm, Variation coefficient of grain size 0.15) | as silver 0.55 |
| Sensitizing dye I | 6.9×10⁻⁵ |
| Sensitizing dye II | 1.8×10⁻⁵ |
| Sensitizing dye III | 3.1×10⁻⁴ |
| Sensitizing dye IV | 4.0×10⁻⁵ |
| EX-2 | 0.350 |
| HBS-1 | 0.005 |
| EX-10 | 0.020 |
| Gelatin | 1.30 |

### Fourth Layer (Second Red Sensitive Emulsion Layer)

### Fifth Layer (Third Red Sensitive Emulsion Layer)

| | |
|---|---|
| Silver iodobromide emulsion (16 mol% AgI, Average grain size 1.1 µm) | as silver 1.60 |
| Sensitizing dye IX | 5.4×10⁻⁵ |
| Sensitizing dye II | 1.4×10⁻⁵ |
| Sensitizing dye III | 2.4×10⁻⁴ |
| Sensitizing dye IV | 3.1×10⁻⁵ |
| EX-13 | 0.005 |
| EX-3 | 0.240 |
| EX-4 | 0.120 |
| HBS-1 | 0.22 |
| HBS-2 | 0.10 |
| Gelatin | 1.63 |

### Sixth Layer (Intermediate Layer)

| | |
|---|---|
| EX-5 | 0.040 |
| HBS-1 | 0.020 |
| Gelatin | 0.80 |

### Seventh Layer (First Green Sensitive Emulsion Layer)

| | |
|---|---|
| Tabular silver iodobromide emulsion (8 mol% AgI, average grain size 0.6 µm, Average aspect ratio 6.0, Average thickness 0.15 µm) | as silver 0.40 |
| Sensitizing dye V | 3.0×10⁻⁵ |
| Sensitizing dye VI | 1.0×10⁻⁴ |
| Sensitizing dye VII | 3.8×10⁻⁴ |
| EX-6 | 0.260 |
| EX-1 | 0.021 |
| EX-7 | 0.030 |
| EX-8 | 0.025 |
| HBS-1 | 0.260 |
| HBS-4 | 0.010 |
| Gelatin | 1.50 |

### Eighth Layer (Second Green Sensitive Emulsion Layer)

### Ninth Layer (Third Green Sensitive Emulsion Layer)

| | |
|---|---|
| Silver iodobromide emulsion (12 mol% AgI, Average grain size 1.0 µm) | as silver 1.2 |
| Sensitizing dye V | 3.5×10⁻⁵ |
| Sensitizing dye VI | 8.0×10⁻⁵ |
| Sensitizing dye VII | 3.0×10⁻⁴ |
| EX-6 | 0.005 |
| EX-13 | 0.007 |
| EX-11 | 0.118 |
| EX-1 | 0.025 |
| HBS-1 | 0.25 |
| HBS-2 | 0.10 |
| Gelatin | 1.74 |

### Tenth Layer (Yellow Filter Layer)

| | |
|---|---|
| Yellow colloidal silver | as silver 0.05 |
| EX-5 | 0.08 |
| HBS-3 | 0.03 |
| Gelatin | 0.95 |

### Eleventh Layer (First Blue Sensitive Emulsion Layer)

### Twelfth Layer (Second Blue Sensitive Emulsion Layer)

| | |
|---|---|
| Mono-disperse silver iodobromide emulsion (14 mol% AgI, Average grain size 0.8µm, Variation coefficient of grain size 0.16) | as silver 0.45 |
| Sensitizing dye VIII | 2.1×10⁻⁴ |
| EX-9 | 0.20 |
| EX-10 | 0.015 |
| HBS-1 | 0.03 |
| Gelatin | 0.46 |

### Thirteenth Layer (Third Blue Sensitive Emulsion Layer)

| | |
|---|---|
| Silver iodobromide emulsion (14 mol% AgI, Average grain size 1.3µm) | as silver 0.77 |
| Sensitizing dye VIII | 2.2×10⁻⁴ |
| EX-9 | 0.20 |
| HBS-1 | 0.07 |
| Gelatin | 0.69 |

### Fourteenth Layer (First Protective Layer)

### Fifteenth Layer (Second Protective Layer)

| | |
|---|---|
| Poly(methyl acrylate) grains (Average diameter about 1.5 µm) | 0.54 |
| S-1 | 0.15 |
| S-2 | 0.05 |
| Gelatin | 0.72 |

The gelatin hardening agent H-1 and surfactant were added to each layer as well as the components indicated above.

### Samples 102 to 117

Samples 102 to 117 were prepared by replacing the couplers in the fifth and ninth layers of Sample 101 with other couplers as shown in Table 1. Here EX-11 was replaced with 0.5 times molar of the other coupler.

These samples were exposed imagewise in such a way as to provide a maximum exposure of 10 CMS using light source A the color temperature of which had been adjusted to 4800°K with filters, after which they were color developed as indicated below.

The color development process was carried out in accordance with the scheme indicated below at a temperature of 38°C.

| | | |
|---|---|---|
| Color Development | 3 minutes | 15 seconds |
| Bleach-A | 6 minutes | 30 seconds |
| Water Wash | 2 minutes | 10 seconds |
| Fix | 4 minutes | 20 seconds |
| Water Wash | 3 minutes | 15 seconds |
| Stabilization | 1 minute | 05 seconds |

The composition of the processing bath used in each process was as indicated below.

### Color Development Bath

| | |
|---|---|
| Diethylenetriamine pentaacetic acid | 1.0 g |
| 1-Hydroxyethylidene-1,1-diphosphonic acid | 2.0 g |
| Sodium sulfite | 4.0 g |
| Potassium carbonate | 30.0 g |
| Sodium bromide | 1.4 g |
| Potassium iodide | 1.3 mg |
| Hydroxylamine sulfate | 2.4 g |
| 4-(N-Ethyl-N-β-hydroxyethylamino)-2-methylaniline sulfate | 4.5 g |
| Water | to make up to 1.0 ℓ pH 10.0 |

### Bleach A Bath

### Fixer Bath

| | |
|---|---|
| Ethylenediamine tetraacetic acid, disodium salt | 1.0 g |
| Sodium sulfite | 4.0 g |
| Aqueous ammonium sulfate solution (70%) | 175.0 ml |
| Sodium bisulfite | 4.6 g |
| Water | to make up to 1.0 ℓ pH 6.6 |

### Stabilizer Bath

| | |
|---|---|
| Formalin (40%) | 2.0 ml |
| Polyoxyethylene p-monononylphenyl ether (average degree of polymerization 10) | 0.3 g |
| Water | to make up to 1.0 ℓ |

Next, development processing was carried out as described above except that the bleach-A bath was replaced by the processing bath indicated below. The bleach-B bath was prepared so as to forcedly simultate a deteriorated bath, i.e., as if the bath had been used to process a large amount of photosensitive material.

The bleach-B bath was prepared by mixing 900 ml of solution (B-1) with 100 ml of solution (B-2).

### Bleach Bath Composition

| | (B-1) | (B-2') |
|---|---|---|
| Ethylenediamine tetraacetic acid, ferric ammonium salt | 90 g | 100 g |
| Ethylenediamine tetraacetic acid, disodium salt | 10 g | |
| Ammonium bromide | 150 g | |
| Ammonium nitrate | 10 g | |
| Aqueous ammonia (27%) | 6.5 ml | |
| Water | to make up to 900 ml | 1 ℓ |

The (B-2) bath was prepared by introducing steel wool into (B-2'), closing the container and leaving the mixture to stand so as to provide a solution in which the Fe(III)-EDTA had been turned into Fe(II)-EDTA.

The decrease in density, when processing photosensitive material in bleach-B bath at an exposure which gave a cyan density of 0.50 on processing in fresh bleach-A bath, is shown in Table 1.

The increase in magenta fog density and the latent image storage properties (reduction in speed at fog+0.2) on leaving samples which had been exposed imagewise in the same way as before and then left to stand for 14 days at a temperature of 40°C, with 80% relative humidity, before being processed using bleach-A bath, is shown in Table 1.

### EXAMPLE 1

Samples 201 to 214 were prepared by replacing the various couplers in the third, fourth, fifth, seventh, eighth and ninth layers of sample 101 as shown in Table 2. Equimolar amounts of the couplers 5, 6, 18 and 19 used in the present invention were used to replace EX-6 in the seventh and eighth layers, and the amounts of HBS-1 and gelatin in the seventh layer were changed to 0.10 and 1.00 respectively while the amount of HBS-1 and gelatin in the eighth layer were changed to 0.08 and 0.80 respectively. Furthermore, coupler 18 used in the present invention was used at a rate of 1/2 molar to replace EX-11 in the ninth layer.

In samples 215 to 218, the HBS-1 in the third and fourth layers of sample 214 was added at a rate of 0.2, 0.4, 0.8 and 1.1 times by weight respectively with respect to A-18, and the amount of gelatin was changed to 1.40, 1.50, 1.65 and 1.80.

These samples were exposed to green light and white light in the same way as in Comparative Example 1, after which they were processed using an automatic developing machine and the method indicated below. (Cumulative replenishment of the bath was carried out to 3 times the tank volume.)

| Operation | Processing Time | | Processing Temperature | Replenishment Rate | Tank Volume |
|---|---|---|---|---|---|
| Color Development | 3 min | 15 s | 38°C | 45 ml | 10 ℓ |
| Bleach | 1 min | 00 s | 38°C | 20 ml | 4 ℓ |
| Bleach-fix | 3 min | 15 s | 38°C | 30 ml | 8 ℓ |
| Rinse (1) | | 40 s | 35°C | Counter-flow pipework from (2) to (1) | 4 ℓ |
| Rinse (2) | 1 min | 00 s | 35°C | 30 ml | 4 ℓ |
| Stabilization | | 40 s | 38°C | 20 ml | 4 ℓ |
| Drying | 1min | 15 s | 55°C | | |

Replenishment rates per 1 meter length×35 mm wide.

The compositions of the processing baths were as follows:

### Color Development Bath

### Bleach Bath Tank=Replenisher

### Bleach-Fix Bath Tank=Replenisher

### Rinse bath Tank=Replenisher

Town water was treated by passing through a mixed bed type column which had been packed with an H-type strongly acidic cation exchange resin ("Amberlite IR-120B", made by the Rohm and Haas Co.) and an OH-type anion exchange resin ("Amberlite IR-400", made by the same company) so as to reduce the calcium and magnesium ion concentrations to less than 3 mg/l, after which 20 mg/l of sodium dichloroisocyanurate and 1.5 g/l of sodium sulfate were added.

The pH of this bath was within the range of from 6.5 to 7.5.

### Stabilization Bath Tank=Replenisher

| | (Units: g) |
|---|---|
| Formalin (37%) | 2.0 ml |
| Polyoxyethylene p-monononylphenylether (average degree of polymerization 10) | 0.3 |
| Ethylenediamine tetraacetic acid, disodium salt | 0.05 |
| Water | to make up to 1.0 ℓ |
| pH | 5.0 - 8.0 |

The relative speeds of the red sensitive layers and green sensitive layers were obtained from processed strips in the same way as in Comparative Example 1. Furthermore, the value obtained by subtracting the yellow fog density from the yellow density at the point at which the magenta density was equal to fog + 1.0 with processed samples which had been exposed to green light are shown as the color turbidity in Table 2.

The samples were exposed to white light with a pattern intended for MTF value measurement purposes, and the MTF value for 25 cycles/mm was obtained with the cyan image.

Moreover, the decreases in density resulting from the utilization of a forcedly fatigued bleach bath were obtained using the same method as in Comparative Example 1.

It is clear from Table 2 that the samples of the present invention exhibited little loss of cyan density on processing in tired baths, gave little color turbidity, and had excellent sharpness as represented by the MTF value.

More specifically, it can be said that Samples 212 to 214 of the present invention exhibit excellent sharpness as represented by MTF value and excellent color reproducibility represented by color turbidity as compared with Samples 101, 201, and 202 for comparison, and little loss of density on processing in the tired bleach-B bath as compared with Samples 101, 203, and 204. From the results of Samples 214 to 218, it can be said that a smaller amount of a high boiling point organic solvent for dispersing the cyan coupler used in the present invention is preferred in view of sharpness.

## Claims

1. A silver halide color photographic material comprising at least two red sensitive silver halide emulsion layers having different speeds and containing at least one cyan coupler;
at least one green sensitive silver halide emulsion layer containing at least one magenta coupler; and
at least one blue sensitive silver halide emulsion layer containing at least one yellow coupler,
wherein said layers are established on a support and at least one of the cyan couplers is represented by the general formula (A), and at least one of the magenta couplers is represented by the general formula (I) or the general formula (II): wherein R₁ represents a halogen atom, an aliphatic group, an aromatic group, a heterocyclic group, an amidino group, a guanidino group or a group which is represented by -COR₄, -SO₂R₄, -SOR₄, -NHCOR₄, -NHSO₂R₄, -HNSOR₄,
R₂ represents a halogen atom, a hydroxyl group, a carboxyl group, a sulfo group, an amino group, a cyano group, a nitro group, an aliphatic group, an aromatic group, a carbonamido group, a sulfonamido group, a carbamoyl group, a sulfamoyl group, a ureido group, an acyl group, an acyloxy group, an aliphatic oxy group, an aromatic oxy group, an aliphatic thio group, an aromatic thio group, an aliphatic sulfonyl group, an aromatic sulfonyl group, an aliphatic sulfinyl group, an aromatic sulfinyl group, an aliphatic oxycarbonyl group, an aromatic oxycarbonyl group, an aliphatic oxycarbonylamino group, an aromatic oxycarbonylamino group, a sulfamoylamino group, a heterocyclic group or an imido group,
1' is 0 or an integer of up to 3,
R₃ represents a hydrogen atom or a R₆U group, T represents a hydrogen atom or a group which can be eliminated by a coupling reaction with the oxidized form of a primary aromatic amine developing agent,
R₄ and R₅ each independently represent an aliphatic group, an aromatic group, a heterocyclic group, an amino group, an aliphatic oxy group or an aromatic oxy group,
R₆ represents a hydrogen atom, an aliphatic group, an aromatic group, a heterocyclic group, a -OR₇ group, a -SR₇ group, a -COR₈ group, a a -PO(R₇)₂ group, a -PO(-OR₇)₂ group, a a a -CO₂R₇ group, a -SO₂R₇ group, a -SO₂OR₇ group or an imido group, and
U represents a 〉N-R₉ group, a -CO- group, a -S0₂- group, a -SO- group or a single bond,
R₇ represents an aliphatic group, an aromatic group or a heterocyclic group,
R₈ represents a hydrogen atom, an aliphatic group, an aromatic group or a heterocyclic group, and
R₉ and R₁₀ each independently represent a hydrogen atom, an aliphatic group, an aromatic group, a heterocyclic group, an acyl group, an aliphatic sulfonyl group or an aromatic sulfonyl group, or may be joined together to form a ring,
when l' has a value of 2 or more, the R₂ groups may be the same or different, or they may be joined together to form a ring, or R₂ and R₃, or R₃ and T, may be joined together to form rings, respectively, or dimers or larger units (oligomers or polymers) can be formed by linking together via divalent groups or groups of higher valence in any of R₁, R₂, R₃ or T,
with the proviso that said cyan coupler of formula (A) is not wherein R₃₁ represents an alkyl group, an aryl group or a heterocyclic group,
R₃₂ represents a hydrogen atom or a substituent group, R₃₂' represents an alkyl group, an aryl group, an alkylthio group, an arylthio group or a heterocyclic thio group, and
X represents a hydrogen atom or a coupling elimination group,
wherein the red sensitive layer having the lowest speed contains a four equivalent cyan coupler of the general formula (A) wherein T is a hydrogen atom and the red sensitive layer having the highest speed contains a two equivalent cyan coupler of the general formula (A) wherein T is a group other than a hydrogen atom.

2. The color photographic material of claim 1, wherein R₁ is selected from the group consisting of a halogen atom, a -COR₄ group and a -SO₂R₄ group, wherein R₄ is an amino group,
1' is 1,
R₂ is selected from the group consisting of a halogen atom, an aliphatic group, an aromatic oxy group, a carbonamido group, a sulfonamido group and a cyano group,
R₃ is a R₆U group, wherein R₆ is selected from the group consisting of an aliphatic group, an aromatic group, a -OR₇ group and an -SR₇ group,
T is selected from the group consisting of a halogen atom, an aliphatic oxy group and an aliphatic thio group,
R₃₂ is selected from the group consisting of an alkyl group, an aryl group, an alkylthio group and an arylthio group, and
X is selected from the group consisting of a halogen atom, a carboxyl group, a group which is linked via an oxygen atom, a group which is linked via a nitrogen atom, and a group which is linked via a sulfur atom.

3. The color photographic material of claim 2, wherein
R₁ is a -COR₄ group, wherein R₄ is an amino group, l₁ is 1,
R₂ is selected from the group consisting of a fluorine atom, a chlorine atom, a trifluoromethyl group, a methoxy group and a cyano group, and
R₃ is selected from the group consisting of an aliphatic oxy carbonyl group, an aliphatic sulfonyl group and an aromatic sulfonyl group.

4. The color photographic material of claim 1, wherein R₃₁ represents an alkyl group or an aryl group.

5. The color photographic material of claim 1, wherein X represents an arylthio group.

6. The color photographic material of claim 1 wherein the amount of a high boiling point organic solvent which is used as a dispersing medium for the coupler represented by formula (I) or (II) is from 0.3 to 1.0 by weight.

7. The color photographic material of claim 1 wherein the amount of a high boiling point organic solvent which is used as a dispersing medium for the coupler represented by formula (A) is from 0 to 0.3 by weight.

## Patentansprüche

1. Farbphotographisches Silberhalogenidmaterial, umfassend
mindestens zwei rotempfindliche Silberhalogenidemulsionsschichten, die unterschiedliche Empfindlichkeiten haben und mindestens einen Cyankuppler enthalten;
mindestens eine grünempfindliche Silberhalogenidemulsionsschicht, die mindestens einen Magentakuppler enthält; und
mindestens eine blauempfindliche Silberhalogenidemulsionsschicht, die mindestens einen Gelbkuppler enthält, worin die Schichten auf einem Träger angeordnet sind und mindestens einer der Cyankuppler dargestellt ist durch die allgemeine Formel (A), und mindestens einer der Magentakuppler dargestellt ist durch die allgemeine Formel (I) oder die allgemeine Formel (II): worin R₁ ein Halogenatom, eine aliphatische Gruppe, eine aromatische Gruppe, eine heterocyclische Gruppe, eine Amidinogruppe, eine Guanidinogruppe oder eine Gruppe, die dargestellt ist durch -COR₄, -SO₂R₄, -SOR₄, -NHCOR₄, -NHSO₂R₄, -HNSOR₄, oder darstellt,
R2 ein Halogenatom, eine Hydroxylgruppe, eine Carboxylgruppe, eine Sulfogruppe, eine Aminogruppe, eine Cyanogruppe, eine Nitrogruppe, eine aliphatische Gruppe, eine aromatische Gruppe, eine Carbonamidogruppe, eine Sulfonamidogruppe, eine Carbamoylgruppe, eine Sulfamoylgruppe, eine Ureidogruppe, eine Acylgruppe, eine Acyloxygruppe, eine aliphatische Oxygruppe, eine aromatische Oxygruppe, eine aliphatische Thiogruppe, eine aromatische Thiogruppe, eine aliphatische Sulfonylgruppe, eine aromatische Sulfonylgruppe, eine aliphatische Sulfinylgruppe, eine aromatische Sulfinylgruppe, eine aliphatische Oxycarbonylgruppe, eine aromatische Oxycarbonylgruppe, eine aliphatische Oxycarbonylaminogruppe, eine aromatische Oxycarbonylaminogruppe, eine Sulfamoylaminogruppe, eine heterocyclische Gruppe oder eine Imidogruppe darstellt,
1' 0 oder eine ganze Zahl bis 3 ist,
R₃ ein Wasserstoffatom oder eine R₆U-Gruppe darstellt,
T ein Wasserstoffatom oder eine Gruppe darstellt, die durch eine Kupplungsreaktion mit der oxidierten Form eines primären aromatischen Amin-Entwicklungsmittels entfernt werden kann,
R₄ und R₅ jeweils unabhängig voneinander eine aliphatische Gruppe, eine aromatische Gruppe, eine heterocyclische Gruppe, eine Aminogruppe, eine aliphatische Oxygruppe oder eine aromatische Oxygruppe darstellen,
R₆ ein Wasserstoffatom, eine aliphatische Gruppe, eine aromatische Gruppe, eine heterocyclische Gruppe, eine -OR₇ -Gruppe, eine -SR₇ -Gruppe, eine -COR₈ -Gruppe, eine - Gruppe, eine -PO(R₇)₂ -Gruppe, eine -PO(-OR₇)₂ -Gruppe, eine -Gruppe, eine -Gruppe, eine -CO₂R₇ -Gruppe, eine -SO₂R₇ -Gruppe, eine -SO₂OR₇ -Gruppe oder eine Imidogruppe darstellt, und U eine 〉N-R₉ -Gruppe, eine -CO- -Gruppe, eine -SO₂- -Gruppe, eine -SO- -Gruppe oder eine Einfachbindung darstellt,
R₇ eine aliphatische Gruppe, eine aromatische Gruppe oder eine heterocyclische Gruppe darstellt,
R₈ ein Wasserstoffatom, eine aliphatische Gruppe, eine aromatische Gruppe oder eine heterocyclische Gruppe darstellt, und
R₉ und R₁₀ jeweils unabhängig voneinander ein Wasserstoffatom, eine aliphatische Gruppe, eine aromatische Gruppe, eine heterocyclische Gruppe, eine Acylgruppe, ein aliphatische Sulfonylgruppe oder eine aromatische Sulfonylgruppe darstellen oder miteinander verbunden sein können, um einen Ring zu bilden, wenn 1' einen Wert von 2 oder mehr hat, die R₂-Gruppen gleich oder verschieden sein können oder miteinander verbunden sein können, um einen Ring zu bilden, oder R₂ und R₃, oder R₃ und T jeweils miteinander verbunden sein können, um Ringe zu bilden, oder Dimere oder größere Einheiten (Oligomere oder Polymere) gebildet werden können durch Verbinden über zweiwertige Gruppen oder Gruppen mit höherer Wertigkeit an irgendeinem von R₁, R₂, R₃ oder T; mit der Maßgabe, daß der Cyankuppler der Formel (A) nicht ist, worin R₃₁ eine Alkylgruppe, eine Arylgruppe oder eine heterocyclische Gruppe darstellt,
R₃₂ ein Wasserstoffatom oder eine Substituentengruppe darstellt,
R₃₂' eine Alkylgruppe, eine Arylgruppe, eine Alkylthiogruppe, eine Arylthiogruppe oder eine heterocyclische Thiogruppe darstellt, und
X ein Wasserstoffatom oder eine bei der Kupplung abspaltbare Gruppe darstellt,
worin die rotempfindliche Schicht mit der geringsten Empfindlichkeit einen Vier-Äquivalent-Cyankuppler der allgemeinen Formel (A) enthält, worin T ein Wasserstoffatom ist, und die rotempfindliche Schicht mit der höchsten Empfindlichkeit einen Zwei-Äquivalent-Cyankuppler der allgemeinen Formel (A) enthält, worin T eine Gruppe ist, die kein Wasserstoffatom ist.

2. Farbphotographisches Material nach Anspruch 1, worin
R₁ gewählt ist aus der Gruppe bestehend aus einem Halogenatom, einer -COR₄ -Gruppe und einer -SO₂R₄ -Gruppe, worin R₄ eine Aminogruppe ist,
l' 1 ist,
R₂ gewählt ist aus der Gruppe bestehend aus einem Halogenatom, einer aliphatischen Gruppe, einer aromatischen Oxygruppe, einer Carbonamidogruppe, einer Sulfonamidogruppe und einer Cyanogruppe,
R₃ eine R₆U-Gruppe ist, worin R₆ gewählt ist aus der Gruppe bestehend aus einer aliphatischen Gruppe, einer aromatischen Gruppe, einer -OR₇ -Gruppe und einer -SR₇ -Gruppe,
T gewählt ist aus der Gruppe bestehend aus einem Halogenatom, einer aliphatischen Oxygruppe und einer aliphatischen Thiogruppe,
R₃₂ gewählt ist aus der Gruppe bestehend aus einer Alkylgruppe, einer Arylgruppe, einer Alkylthiogruppe und einer Arylthiogruppe, und
X gewählt ist aus der Gruppe bestehend aus einem Halogenatom, einer Carboxylgruppe, einer Gruppe, die über ein Sauerstoffatom verbunden ist, einer Gruppe, die über ein Stickstoffatom verbunden ist und einer Gruppe, die über ein Schwefelatom verbunden ist.

3. Farbphotographisches Material nach Anspruch 2, worin
R₁ eine -COR₄ -Gruppe ist, worin R₄ eine Aminogruppe ist,
l₁ 1 ist,
R₂ gewählt ist aus der Gruppe bestehend aus einem Fluoratom, einem Chloratom, einer Trifluormethylgruppe, einer Methoxygruppe und einer Cyanogruppe, und
R₃ gewählt ist aus der Gruppe bestehend aus einer aliphatischen Oxycarbonylgruppe, einer aliphatischen Sulfonylgruppe und einer aromatischen Sulfonylgruppe.

4. Farbphotographisches Material nach Anspruch 1, worin R31 eine Alkylgruppe oder eine Arylgruppe darstellt.

5. Farbphotographisches Material nach Anspruch 1, worin X eine Arylthiogruppe darstellt.

6. Farbphotographisches Material nach Anspruch 1, worin die Menge eines organischen Lösungsmittels mit hohem Siedepunkt, welches als Dispergiermittel für den durch Formel (I) oder (II) dargestellten Kuppler verwendet wird, 0,3 bis 1,0, bezogen auf das Gewicht, beträgt.

7. Farbphotographisches Material nach Anspruch 1, worin die Menge eines organischen Lösungsmittels mit hohem Siedepunkt, welches als Dispergiermittel für den durch Formel (A) dargestellten Kuppler verwendet wird, 0 bis 0,3, bezogen auf das Gewicht, beträgt.

## Revendications

1. Matériau photographique couleur à l'halogénure d'argent comprenant :
au moins deux couches d'émulsion à l'halogénure d'argent sensible au rouge ayant différentes vitesses et contenant au moins un coupleur pour le cyan ;
au moins une couche d'émulsion à l'halogénure d'argent sensible au vert contenant au moins un coupleur pour le magenta ; et
au moins une couche d'émulsion à l'halogénure d'argent sensible au bleu contenant au moins un coupleur pour le jaune, où lesdites couches sont établies sur un support et au moins l'un des coupleurs pour le cyan est représenté par la formule générale (A), et au moins l'un des coupleurs pour le magenta est représenté par la formule générale (I) ou la formule générale (II) : où
R₁ représente un atome d'halogène, un groupe aliphatique, un groupe aromatique, un groupe hétérocyclique, un groupe amidino, un groupe guanidino ou un groupe qui est représenté par : -COR₄, -SO₂R₄, -SOR₄, -NHCOR₄, -NHSO₂R₄, -HNSOR₄, ou
R₂ représente un atome d'halogène, un groupe hydroxyle, un groupe carboxyle, un groupe sulfo, un groupe amino, un groupe cyano, un groupe nitro, un groupe aliphatique, un groupe aromatique, un groupe carbonamido, un groupe sulfonamido, un groupe carbamoyle, un groupe sulfamoyle, un groupe uréido, un groupe acyle, un groupe acyloxy, un groupe oxy aliphatique, un groupe oxy aromatique, un groupe thio aliphatique, un groupe thio aromatique, un groupe sulfonyle aliphatique, un groupe sulfonyle aromatique, un groupe sulfinyle aliphatique, un groupe sulfinyle aromatique, un groupe oxycarbonyle aliphatique, un groupe oxycarbonyle aromatique, un groupe oxycarbonylamino aliphatique, un groupe oxycarbonylamino aromatique, un groupe sulfamoylamino, un groupe hétérocyclique ou un groupe imido,
l' est 0 ou un entier pouvant atteindre 3,
R₃ représente un atome d'hydrogène ou un groupe R₆U,
T représente un atome d'hydrogène ou un groupe qu'on peut éliminer par une réaction de couplage avec la forme oxydée de l'agent développateur amine aromatique primaire,
R₄ et R₅ représentent chacun indépendamment un groupe aliphatique, un groupe aromatique, un groupe hétérocyclique, un groupe amino, un groupe oxy aliphatique ou un groupe oxy aromatique,
R₆ représente un atome d'hydrogène, un groupe aliphatique, un groupe aromatique, un groupe hétérocyclique, un groupe -OR₇, un groupe -SR₇, un groupe -COR₈, un groupe un groupe -PO(R₇)₂, un groupe -PO(-OR₇)₂, un groupe un groupe un groupe -CO₂R₇, un groupe -SO₂R₇ un groupe -SO₂OR₇ ou un groupe imido, et U représente un groupe 〉N-R₉, un groupe -CO-, un groupe -SO₂-, un groupe -SO- ou a une liaison simple,
R₇ représente un groupe aliphatique, un groupe aromatique ou un groupe hétérocyclique,
R₈ représente un atome d'hydrogène, un groupe aliphatique, un groupe aromatique ou un groupe hétérocyclique, et
R₉ et R₁₀ représentent chacun indépendamment un atome d'hydrogène, un groupe aliphatique, un groupe aromatique, un groupe hétérocyclique, un groupe acyle, un groupe sulfonyle aliphatique ou un groupe sulfonyle aromatique, ou on peut les lier pour former un cycle,
quand 1' a la valeur de 2 ou plus, les groupes R₂ peuvent être identiques ou différents, ou on peut les relier ensemble pour former un cycle, ou R₂ et R₃, ou R₃ et T, peuvent être liés ensemble pour former des cycles, respectivement, ou des dimères ou des unités plus importantes (oligomères ou polymères) peuvent être formés en les reliant par des groupes divalents ou des groupes de valence supérieure dans l'un quelconque des groupes choisis parmi R₁, R₂, R₃ ou T; à la condition que ledit coupleur pour le cyan de la formule (A) n'est pas où
R₃₁ représente un groupe alkyle, un groupe aryle ou un groupe hétérocyclique,
R₃₂ représente un atome d'hydrogène ou un groupe substituant,
R_{32'} représente un groupe alkyle, un groupe aryle, un groupe alkylthio, un groupe arylthio ou un groupe thiohétérocyclique, et
X représente un atome d'hydrogène ou un groupe d'élimination de couplage,
où la couche sensible au rouge ayant la vitesse la plus lente contient un coupleur pour le cyan à quatre équivalents de la formule générale (A) où T est un atome d'hydrogène et la couche sensible au rouge qui a la vitesse la plus rapide contient un coupleur pour le cyan à deux équivalents de formule générale (A) où T est un groupe différent d'un atome d'hydrogène.

2. Matériau photographique couleur selon la revendication 1,
où R₁ est choisi dans le groupe constitué d'un atome d'halogène, d'un groupe -COR₄ et d'un groupe -SO₂R₄, où R₄ est un groupe amino,
l' est 1,
R₂ est choisi dans le groupe constitué d'un atome d'halogène, d'un groupe aliphatique, d'un groupe oxy aromatique, d'un groupe carbonamido, d'un groupe sulfonamido et d'un groupe cyano,
R₃ est un groupe R₆U, où R₆ est choisi dans le groupe constitué d'un groupe aliphatique, d'un groupe aromatique, d'un groupe -OR₇ et d'un groupe -SR₇, T est choisi dans le groupe constitué d'un atome d'halogène, d'un groupe oxy aliphatique et d'un groupe thio aliphatique,
R₃₂ est choisi dans le groupe constitué d'un groupe alkyle, d'un groupe aryle, d'un groupe alkylthio et d'un groupe arylthio, et
X est choisi dans le groupe constitué d'un atome d'halogène, d'un groupe carboxyle, d'un groupe qui est fixé par l'intermédiaire d'un atome d'oxygène, d'un groupe qui est fixé par l'intermédiaire d'un atome d'azote, et d'un groupe qui est fixé par l'intermédiaire d'un atome de soufre.

3. Matériau photographique couleur selon la revendication 2, où
R₁ est un groupe -COR₄, où R₄ est un groupe amino, l₁ est 1,
R₂ est choisi dans le groupe constitué d'un atome de fluor, d'un atome de chlore, d'un groupe trifluorométhyle, d'un groupe méthoxy et d'un groupe cyano, et
R₃ est choisi dans le groupe constitué d'un groupe carbonyloxy aliphatique, d'un groupe sulfonyle aliphatique et d'un groupe sulfonyle aromatique.

4. Matériau photographique couleur selon la revendication 1, où R₃₁ représente un groupe alkyle ou un groupe aryle.

5. Matériau photographique couleur selon la revendication 1, où X représente un groupe arylthio.

6. Matériau photographique couleur selon la revendication 1, où la quantité de solvant organique à haut point d'ébullition qu'on utilise comme milieu dispersant du coupleur représenté par la formule (I) ou (II) représente 0,3 à 1,0 en poids.

7. Matériau photographique couleur selon la revendication 1, où la quantité de solvant organique à haut point d'ébullition qu'on utilise comme milieu dispersant du coupleur représenté par la formule (A) représente 0 à 0,3 en poids.
